

[54] METHOD OF COAL WASHING AT LOW SPEED PUMPING

[76] Inventor: Delbert I. Liller, Rte. 4, Box 64, Deer Park, Md. 21550

[21] Appl. No.: 158,250

[22] Filed: Jun. 10, 1980

## Related U.S. Application Data

[62] Division of Ser. No. 63,707, Aug. 6, 1979, abandoned.

[51] Int. Cl.<sup>3</sup> ..... B02C 19/12

[52] U.S. Cl. ..... 241/21; 241/24; 209/3; 209/211

[58] Field of Search ..... 209/144, 211, 3, 13, 209/12; 220/327, 328; 210/812 R, 812 M; 285/286, 102; 241/20, 24, 21; 137/561 A, 861

## [56] References Cited

## U.S. PATENT DOCUMENTS

|            |         |          |           |
|------------|---------|----------|-----------|
| Re. 56,120 | 11/1909 | Visman   | 209/211   |
| 1,215,890  | 2/1917  | Thuneman | 209/144   |
| 1,309,879  | 7/1919  | Davids   | 209/144 X |
| 2,288,297  | 6/1942  | Naiman   | 137/561 A |
| 2,522,217  | 9/1950  | Tacohus  | 285/286   |
| 2,816,658  | 12/1957 | Braun    | 210/512 R |
| 2,885,223  | 5/1959  | Duff     | 285/402 X |
| 2,967,618  | 11/1961 | Vane     | 210/512 R |
| 3,033,145  | 5/1962  | Thielsch | 285/286   |
| 3,082,645  | 4/1963  | Eddy     | 209/211   |
| 3,126,160  | 3/1964  | Beiger   | 285/401 X |
| 3,136,723  | 6/1964  | Erwin    | 210/512 R |

|           |         |           |             |
|-----------|---------|-----------|-------------|
| 3,172,844 | 8/1965  | Kurz      | 209/149 X   |
| 3,198,560 | 8/1965  | Collins   | 285/280     |
| 3,800,946 | 4/1974  | Reid      | 210/512 R X |
| 3,887,456 | 6/1975  | Loughner  | 209/211     |
| 3,897,609 | 8/1975  | Schmidt   | 220/327     |
| 3,901,799 | 8/1975  | Adkison   | 299/144     |
| 3,902,601 | 9/1975  | Townley   | 209/211 X   |
| 3,923,210 | 12/1975 | Alexander | 210/512 R   |
| 4,090,956 | 5/1978  | Benson    | 210/512 R   |
| 4,226,708 | 10/1980 | McCartney | 209/211     |

## OTHER PUBLICATIONS

Min Eng., Mar. 1953, pp. 304-308, Operating Behavior of Liquid-Solid Cyclone, Fitch et al.

Primary Examiner—Robert Halper  
Attorney, Agent, or Firm—Abraham A. Saffitz

## [57] ABSTRACT

A method of coal washing at low speed pumping using a centrifugal cyclone of circular cross section having a bowl of diameter B and fitted with a vortex finder, a vortex finder sleeve, a dish, an orifice at the bottom and an inlet near the top in which a critical geometry is provided for the dish as part of a one-piece orifice dish unit so that the recovery of coal can be adjusted at low pumping speed of the water entering the inlet. The pumping speed may vary from 6 to 16 feet of water per second under a pressure of 8 to 15 psig. The orifice dish unit is made of a specified abrasion resistant material.

5 Claims, 25 Drawing Figures







Fig. 5



Fig. 7



Fig. 6



Fig. 8





Fig. 12



Fig. 13



Fig. 14



Fig. 17



Fig. 18



Fig. 19



Fig. 16

Fig. 20

Fig. 21



ASH REMOVAL  
 $3/4 \times 0$  FEED



Fig. 23.

INORGANIC SULFUR REMOVAL  
 $3/4 \times 0$  FEED



Fig. 24.



## METHOD OF COAL WASHING AT LOW SPEED PUMPING

This is a division, of application Ser. No. 063707, filed 5 Aug. 6, 1979 now abandoned.

### CROSS REFERENCE TO RELATED APPLICATIONS

| Case No. | Title                                                                                                                                                                        |
|----------|------------------------------------------------------------------------------------------------------------------------------------------------------------------------------|
| 3-I      | Construction Of Shallow Dish With Tapered Orifice For Streamlined Flow Cyclone Washing Of Crushed Coal; Serial No. 2,731, filed January 11, 1979 now U.S. Pat. No. 4,224,143 |
| 3-II     | Adjustable Vortex Finder; Serial No. 56,109, filed July 9, 1979, now abandoned                                                                                               |
| 3-III    | Method Of Installing Replaceable Sleeve In Fixed Vortex Finder; Serial No. 56,108, filed July 9, 1979 now U.S. Pat. No. 4,235,363                                            |

10 20 30 35 40 45 50 55 60 65

### BACKGROUND OF THE INVENTION

#### FIELD OF THE INVENTION

This invention lies in the field of washing coal with water only in a shallow bottomed centrifugal separating cyclone of circular cross-section having a cylindrical portion with a diameter to height ratio of 0.8 to 1.3, preferably 0.90 to 0.95, the cyclone fitted with a single inlet pipe, a shallow dish below the cylindrical portion, a single bottom orifice fitted to the shallow dish and a fixed vortex finder leading to an outlet at the top for removal of washed coal. Gravity separation under streamlined flow is accomplished with light coal particles at a gravity value down to about 1. using crushed coal ranging in size from  $1\frac{1}{4}'' \times 0$  down to  $\frac{3}{8}'' \times 0$ . 25

The invention also lies in the field of providing an easily insertable abrasion resistant separator bottom having unique toughness and wear resistance characteristics to provide trouble-free, efficient coal washing based on the special material characteristics and the critical geometry of the shallow bottom dish which adapts it to fit in a closely contoured relationship to the cylindrical portion of the cyclone. 30

The invention deals with minimal water to the pumps and separators while separating heavy solids from light solids in centrifugal cyclone gravity separation. 45

Further, the invention lies in the field of rebuilding cyclones to include the insertable dish and orifice and set the critical adjustments of the invention. 50

The invention also lies in the field of cleaning ores other than coal to rid them of impurities by taking advantage of the newly discovered efficiency and capacity taught in the present application. 55

In particular, the field of the invention is that of my Case No. 1, Ser. No. 860,330, filed Dec. 14, 1977, now U.S. Pat. No. 4,219,409, but added to Case No. 1 teachings are the empirically determined critical values above identified to extend the use of the invention to greater efficiency and economy to meet the operating requirements for cleaning of any commercially producible coal with water only and to reduce its non-combustible ingredients prior to using the coal in a utility or steel plant, in a pipeline for transportation or for industrial or home heating. 60

The invention also deals with ecology in washing raw coal to get clean coal while removing refuse, this eliminating cancer causing materials and other pollutants. 65

Similarly, cancer causing asbestos is removed from taconite. Cancer inducing fly ash by the test for "bacteria mutation" is removed from the coal before burning.

### COMMERCIAL CYCLONES

The least expensive way to deal directly with the impurities that pollute the environment is to remove them in a water washing centrifugal cyclone machine, such as a hydrocyclone. In 1977 there were 177 coal companies using hydrocyclones, as listed in the *Keystone Coal Industry Manual*. The basic cyclone design has not changed in many years and, apart from the invention in Case No. 1 for streamlined flow in a short space by turning the material twice around before entering the cyclone dish zone, there has been no major change in the prior art. 15

### ENERGY POLICY FOR SWITCHING FROM OIL TO COAL

Since the energy requirement for pollution control is mandatory for all utilities burning coal to generate electrical power, it is obvious that any efficient system to remove mineral ash and sulfur from coal will benefit the public, save money and minimize respiratory risk from steam generating plants, see *Fortune*, Nov. 20, 1978, pages 50 through 60. It is equally obvious that removal of inorganic sulfur from the coal by efficient washing will save substantial maintenance costs for expensive pollution control equipment which the utilities are now required to install. Accordingly, serious attention is merited for preparing freshly mined coal prior to using it. It is elementary good sense to wash coal and remove likely respiratory disease-causing chemicals, e.g.,  $\text{SO}_2$  and fly ash, rather than to burn dirt at a steel plant or utility. Preparation costs are rising, mainly due to the increased costs for large capital outlays for jigging equipment. 20 30 35 40 45 50 55 60 65

### DESCRIPTION OF THE PRIOR ART

#### 1. Copending Application Ser. No. 860,330, filed Dec. 14, 1978:

My copending application, Case No. 1, Ser. No. 860,330, filed Dec. 14, 1977, is incorporated herein by reference and teaches creating directed streamlined flow by directing incoming high solids concentrations of crushed coal in water tangentially along the wall of the bowl of a shallow bottomed cyclone while diverging two streams, namely the incoming inlet coal slurry stream and the swirling coal slurry stream, in the cyclone. As a result, the essential preliminary condition of streamlined flow is created. This flow must occur in the centrifugal cyclone in order to accomplish efficient and high capacity washing of coal or other ores to separate impurities having a different gravity than the cleaned material. 50

#### 2. Prior literature on Operation of Centrifugal Separating Cyclones:

*Chemical Engineers' Handbook* by Robert H. Perry and Cecil H. Chilton, published by McGraw-Hill Book Company, at pages 21 through 57 describes the operating conditions for the separating cyclone water washing of coal, namely inlet pressure of about 10 to 14 pounds per square inch gauge pressure for a 20 to 24 inch cyclone, which is the commonly used cyclone size in coal washing plants. The lower limit below which recovery of low gravity coal cannot be achieved is about 6 to 8

pounds per square inch gauge pressure. Finer sizes of crushed coal are separated at slightly higher pressures but pressures above 14 pounds per square inch are not recommended because of accelerated water. Residence time is very short. The cyclone shown in the Handbook has a long cone and a large volume is circulated for each ton of feed treated in the cone. This results in high energy consumption, low tonnage recovery based on water used and high equipment cost.

Coal Processing Equipment of Uniontown, Pennsylvania describes a Var-A-Wall coal washing plant in the brochure entitled "Hydronomic Modular, Multimedia Coal Washer". The Coal Processing Equipment plant is designed to provide an outside adjustable wall to increase the height of the cyclone. The dominant feature is jiggling with washing done under low water pressure. The extension of the cylinder wall length and volume and a variable depth adjustment of the vortex finder tube create a higher energy loss in a longer cyclone with greater water requirements.

*The Keystone Coal Industry Manual*, Copyright 1977, McGraw-Hill, Inc., is a directory of mechanical coal cleaning plants which describes the name, location, daily capacity, type of cleaning and plant design. The directory identifies 175 plants within the continental United States and 2 plants in Canada which use low pressure jiggling cyclones for coal washing at low solids. Most of these jiggling cyclones are heavy media plants utilizing a magnetite suspension. Substantially all heavy media cyclones operate at recommended 10 to 12 pounds per square inch pressure. Present recommendations to coal plant operators is to utilize jiggling action and steeper cones so that the pressure drops in the cone substantially to atmospheric pressure at the refuse outlet.

The article "Preparation Trends" published in *World Coal*, March 1978, page 13, gives the basic performance data for a heavy media jiggling cyclone (24 inch). The crushed coal feed is  $\frac{3}{8}'' \times 0$  which is separated in three fractions, e.g.,  $\frac{3}{8}'' \times 28$  mesh, 28 mesh  $\times 100$  mesh and 100 mesh  $\times 0$ . These plants operate at a 1.76 density separation. Magnetite losses are about 1 kilogram per ton of coal washed. The objective is for a separation as low as 1.40 relative density.

The Jan. 1, 1978 issue of *Coal Age*, pages 65 through 84, provides a portfolio of flow sheets for the washing plant at the American Electric Power Mine, Helper site, Salt Lake City, Utah using heavy media cyclones and special water conservation methods. A similar heavy media plant is shown of the Roberts and Schaefer design with a production rate of 1,750 tons per hour. A third heavy media plant from McNally-Pittsburgh is shown for the Jefferson County Mine in Alabama. Still another heavy media Heyl and Patterson cyclone plant is shown which is designed for existing 650 Mw generating units. Yet another preparation plant is shown in Mingo County, West Virginia. All of these use heavy media and all are in the multi-million dollar category. In contrast, the capital investment in the present retrofitted cyclone is a small fraction of these costs. To illustrate, the McNally-Pittsburgh plant at Wilson, Maryland invested 96 million dollars to process 1,000 tons per hour by jiggling while the two stage plant of the invention invests slightly less than 1 million dollars to process 150 tons per hour by streamlined centrifugal separation. At the same output, the jiggling choice costs 15 times as much as the centrifugal separation of the invention.

As reported in *The New York Times* on Feb. 10, 1978, the Coal Policy Project which was organized in 1976 under the sponsorship of the Center for Strategic and International Studies at Georgetown University, Washington, D.C. has brought agreement on more than 200 steps to help the nation switch from oil to coal in ways that are economically sound and environmentally tolerable. One main recommendation was that producible coal, e.g., coal which is more than 50% coal content and less than 50% impurity (United States Geological Survey definition), should be mined in those parts of the country where the product will have the highest heat content. Further, agreement was reached that Eastern coal is more efficient and cleaner, in terms of pollution, than Western coal. Deep underground mining in Southern Illinois, Indiana and the Appalachian states was recommended. Strip mining was thought best confined to only thick seams in Wyoming. All parties agreed that costs of electrical energy should be kept down, research on removing dirt should be stepped up, transportation should be improved and washing technology encouraged.

3. Prior Art in The United States Patent Office:

a. Water Only Coal Washing Operations:

Fitch, U.S. Pat. No. 2,981,413, dated Apr. 1961, proposed the use of a vortex finder as a classifier means in a large capacity cyclone for the separation of fine from coarse particles in a process of separating solids in liquid suspension.

Visman, Reissue 26,720, dated November 1969, was the first to realize success in keeping size separation, as in Fitch, to a minimum while achieving gravity separation using finely crushed coals. Visman's examples are all at  $\frac{1}{4}'' \times 0$  at low pulp solids at about 10% in contrast to 10% to 35% of solids herein. Visman's object was to achieve a jiggling action along a horizontal section of his uniquely designed cyclone to separate fine particles from coarse particles in contrast to centrifugal separation herein. Both Visman and Fitch first created turbulence by jiggling and then tried to control turbulence at the separation zone where the light particles were removed from the heavy particles. In contrast, the invention herein described avoids turbulence.

Loughner, U.S. Pat. No. 3,887,456, dated June 1975, discloses a shallow bottomed separating cyclone in which controlled turbulence by jiggling is introduced into the bowl by riffler means. In Loughner, rifflers are provided to gently open a bed of heavier particles and release lighter particles, thereby permitting the lighter particles to be displaced and more centrally aligned for more complete separation.

Samson et al, U.S. Pat. No. 2,377,524, dated June 1945, is cited by Fitch in his U.S. Pat. No. 2,981,413 as an early example of an unobstructed freely whirling liquid in the interior of the casing having an axis of radial symmetry, the casing fitted with a vortex finder for clean particles at the top and an orifice at the bottom through which the heavy particles of grit and sand are removed. Samson emphasized the high velocity of 25 feet per second which sets up centrifugal separating forces to push heavy particles against the wall of the cone creating a vortical whirl which causes an upward stream of lights at the center of the cone. Both Fitch and Samson teach a long cone dimension, in Samson 5 to 15 times the diameter of the cylindrical portion, leading one away from the shallow dish concept of the present invention.

In contrast, Visman and Loughner teach a shallow cone in which the cone height is far less than the diameter of the cylindrical portion and in which the orifice structure has either no taper (purely cylindrical) or only a slight taper, but each seeks turbulence by gentle jiggling at the bottom.

Only Fitch and Samson are high velocity operations, e.g., about 25 feet per second, which is between 310 and 320 rpm, while Loughner and Visman are low velocity operations, e.g., less than half the velocity of Fitch and Samson.

Dehne, U.S. Pat. No. 3,802,570, dated April 1974, is cited to show a special type of orifice construction to prevent reentrainment of heavy particles into the cleaned particles stream at the center of the swirling vortex. Dehne teaches that the major serious problem with efficiency caused by reentrainment occurs in the region of the exit from the conical housing out of the lower orifice of the discharge outlet. A special construction for stabilization is provided of steel or corrosion resistant material for the ascending stream.

b. Erosion Resistant Separable Dishes In The Form Of Linings Or Moldings:

Hirsch, U.S. Pat. No. 2,975,896, dated March 1961, describes the basic construction of a three piece cyclone, e.g., a top cylindrical portion bolted to an intermediate conical portion which is in turn bolted to a bottom tapered orifice portion. Hirsch recognized that the tapered dish constituting the intermediate portion and the orifice portion would wear faster, necessitating replacement of the worn part.

Eddy et al, U.S. Pat. No. 3,087,896, dated April 1963, emphasized the abrasion resistant lining material provided in the easily erodible parts, namely the cone and orifice, and suggested coating of tungsten carbide and alumina as examples of material for lining steel.

Erwin et al, U.S. Pat. No. 3,136,723, dated June 1964, is similar to Eddy but uses an apertured plate to support the cone bolted to the cylindrical portion.

Other linings, much softer than tungsten carbide, have been suggested for the easily erodible conical parts and orifice structures, e.g., cured urethane rubber which is cast onto the fabricated steel cone in Feasel, U.S. Pat. No. 3,499,531, dated March 1970. The rubbers are less desirable than ceramic but more desirable than steel.

Townley, U.S. Pat. No. 3,902,601, dated September 1975, improved these abrasion resistant properties of the cyclone cone with a one piece molded polyurethane rubber cone combined with an orifice to bolt onto a urethane lined cylindrical portion, e.g., a two piece cyclone without the use of any plate supports.

c. Visman Geometry Versus Liller Geometry:

The Visman angle of 135° compared to about 35° for Liller's first included angle in the dish causes too fast an expansion on the helical path of the swirling slurry, not allowing sufficient time for the first layer directing force to be applied to the different specific gravity particles. The large angle causes a high degree of remixing of the high specific gravity particles with the low specific gravity particles via turbulence.

Visman goes from a B" diameter to a 0.42 B" diameter in 0.11 B" of verticle height compared to Liller going from a B" diameter to 0.4 B" diameter in 0.2 B" of vertical height. Visman's bottom is a low centrifugal force turbulent flow jiggling bottom. Liller's bottom is a high centrifugal force streamlined flow smooth bottom. The flow path turn is much too fast in Visman.

The turbulence created when using Visman's bottom in a high centrifugal force, high flow cyclone would destroy all laminar flow created, thus completely breaking down the centrifugal particle separating zone by specific gravity which results in a very poor quality clean coal. Separating efficiency is lost under turbulence.

Visman's bottom is very similar to Loughner's bottom, going from a straight wall to a very flat surface in a short vertical distance.

It is noted that FIG. 3 on sheet 1 of Visman's patent does not agree with FIG. 1 on the same sheet, thus indicating that a different scale was used.

From my experience in the plant with recovery, in Visman's FIG. 1 geometry the recoveries obtained were in the range of 70% to 95%. By changing the geometry to that of FIG. 3, the recoveries are lowered by approximately 50%.

Using either of the above Figs. produces a very low efficiency separation process compared to streamlined centrifugal force cyclone operation.

Visman

1. Operates under back pressure;
2. Lower end of vortex finder is located a predetermined distance between the first and second conical portions; drawing shows location at top of dish section;
3. Conical frustum (included angle faces) of increasing inclination toward the open aperture;
  - a. First conical angle frustum greater than 100° and of the order of 135°;
  - b. Second conical frustum of the order of 75°;
  - c. Third conical frustum of the order of 20°;
4. Separation:
  - a. Coarse particles separate in conical section 19;
  - b. Middlings separate in conical section 20;
  - c. Fines separate in conical section 21.
- d. Critical Wear and Geometry:

Day, U.S. Pat. No. 4,053,393, states at column 1, lines 50 through 57, that the main problem of a replaceable rubber or ceramic liner or composite abrasion resistant liner is the wearing at the smaller diameter parts. Day acknowledges that others, such as Erwin et al and Gilbert, have partly overcome the problem by combining ceramic with molded rubber parts to put the ceramic in the greatest zone of wear but that this requires a fit between rubber and ceramic parts to prevent leakage and interference with proper flow, which is essential in producing the separation of lighter particles from heavier particles.

Criner, U.S. Pat. No. 2,622,735, and Townley, U.S. Pat. No. 3,902,601, were found by Day to be inadequate because of small part movement in the downward direction even though movement in the upward direction was prevented by the shoulder in the shell.

Samson, U.S. Pat. No. 2,377,524, teaches continuously separating solid material, such as grit or sand which is heavier than the product pulp which is being continuously recovered, at a pulp flow of 18 gallons per minute in a whirling motion at 0.5% pulp solids content. The cyclone has a very short cylindrical section (2" to 4") and a long conical portion, with a cylindrical portion of about 33" in length in axial alignment to the outlet. The bottom of the cone has a diameter of  $\frac{1}{8}$  to  $\frac{1}{4}$  of the cylindrical portion. Samson emphasized that the interior of the cyclone must be smooth and absolutely free of any rough projection that would cause turbu-

lence or flow retardation, e.g., at sharp corners or abrupt curvature changes.

Samsom also stressed that a high velocity of 25 feet per second created a vortex or vortical whirl and set up a centrifugal force that would separate particles that are slightly higher in gravity than the pulp and forced the heavy particles out against the wall of the cone while the light pulp particles, which are affected less by centrifugal action, stayed at the inside. Simultaneously, the vortical whirl caused an upward whirling moving stream at the center of the chamber lying within the downwardly moving whirling stream.

The long cone dimension, 5 to 15 times the cylindrical dimension, which Samson stressed created a removal zone in the cone and precluded any friction creating projections to attain the removal of 97% of the dirt in the downward continuously exiting stream and the recovery of the washed pulp in the continuously drawn upward stream. To treat 5 parts of pulp on a dry basis, 995 parts of water is required in Samson at a feed intake of 18 gallons per minute, which corresponds to 25 feet per second.

It would be expected that, if 995 parts of water can remove 97% of the dirt associated with 0.5% solids in a deep cone cyclone, then a lesser ash removal would be achieved with a shallow cylindrical portion and a shorter conical section relative to the height of the cylindrical portion.

Thus, if 800 parts of water and 200 parts of solids were used, as in the invention, a 400 fold increase of 30 solids, one would expect possible half of the mineral ash, sand and grit removal as in Samson.

The soft and flexible material making up the small liner part in Criner and Townley causes intolerable independent movement of the lower end of the liner part and thereby interrupts the smooth surface over which flow takes place. See lines 6 through 26 in Day.

The following discoveries concerning erosion of the small lining parts in Day et al, U.S. Pat. No. 4,053,393, have been made after washing hundreds of thousands of 40 tons of coal:

1. Parting line between the small liner part (orifice) and the large liner part (dish) changes the flow pattern at the printing line and accelerates wear in both directions, up and down;

2. Dimensions of thickness worn away may be controlled within a specific geometric curved pattern in both zones, one upstream and one downstream of the parting line;

3. This control of the zone is based only on the compound curvature of the larger part (dish), the compound curvature of the smaller part (orifice) and a smooth uninterrupted unique compound curvature between upper and lower parts.

In each of the above three discoveries, the interior 55 surface of the dish blended smoothly with the interior surface of the cylindrical portion of the cyclone in which the inlet was fitted. In contrast to the cemented dish construction of jiggling cyclones, such as described in Lougner, U.S. Pat. No. 3,887,456, dated June 1975, the one piece dish-orifice unit of the present invention is not cemented.

In order to apply these discoveries in practical engineering terms, it was found that all dimensions of the cyclone, vortex finder and dish must be expressed in 65 terms of the cyclone bowl inside diameter B whereby the results determined for one size cyclone diameter can be accurately predicted for another size, e.g., in diameter

ter changing from an 18" to a 20" diameter or to a 14" diameter of B. These cyclone dimensions are shown in Table A herein.

4. Commercial Water Only Jigging Cyclones for Separating Low Grade Coal From Refuse (See Lougner U.S. Pat. No. 3,887,456

#### a. Operating Velocities and Pressures

Water only jigging cyclones are the most recent centrifugal machines used to recover usable low grade steam coal from gob or refuse in the usual cleaning plants or at the mine.

The jigging cyclones are adjusted to process high mineral ash raw product having values of 30 to 50% mineral ash at a 1.65 specific gravity separation range.

The feed varies from 20 to 50 TPH of raw coal requiring a pumping capacity from 600 to 1900 GPM of coal water slurry. These feed rates permit either low or high cyclone pressures and fluid velocities, e.g., pressures from 8 to 25 psi and fluid velocities from 10 to 22 feet per second.

However, the operator adjusts the velocity and pressure to maximize the percent recovery (the amount of product reporting out through the vortex finder being preferably 70% of the inlet feed entering the cyclone. Adjustment is made by changing the vortex finder depth and the diameter of the apex in the refuse outlet.

By further trial and error, one can further adjust the recovery for better quality of product. Since jigging cyclones require turbulence while centrifugal separating cyclones have impaired efficiency under turbulence. Hence, an optimum operating efficiency value is different for each type of cyclone and each has very different optimum capacity.

Since the efficiency values for the jigging cyclone depends upon the relative amount of mineral ash, pyritic sulphur, and other impurities, it is usually preferred to go to lower velocities and by combining jigs, float-sink tanks, and other separating devices, the design engineer can plan for as many separating stages as are necessary to obtain the optimum recovery and coal quality as predicted by a laboratory float sink test of the raw coal sample, whether it be taken from a refuse pile, strip coal, deep mined coal, hard coal, soft coal, crop coal, or fully developed nonoxidized coal.

Although the jigging cyclone worked well on raw coals that could be washed for separation of 1.65 gravity and above, it soon became evident that separation below 1.65 gravity could not be achieved and only low quality steam coal was recovered. Typical results in the jigging cyclone were as follows:

Raw coal feed rate—20 to 50 TPH

% solids—5% to 12%

% recovery—25 to 40% (Refuse thrown away 60% to 75%)

Best Quality Product—low quality steam coal

5. Unsuccessful Experiments with Jigging Cyclones

#### a. Settings of Jigging Cyclone

At settings of jigging cyclone of 1.65 and above, the first changes tried were to lower the specific gravity by means of greater constant pumping pressure including the following steps of adjustment; raise vortex finder and widen orifice diameter to overcome turbulent flow.

The velocity was increased from 8 feet per second to 17 feet per second. The results showed no change in coal density from the specific gravity change attempted. At the higher fluid velocities the raw coal feed rate increased from 30 to 45 TPH to unsuccessfully attempt improvement of higher solids being processed.

The results were no better at higher solids or at higher velocities and the turbulence increased.

The next unsuccessful adjustment attempted was varying the vortex finder depth and observing the percent recovery and specific gravity of the cleaned product. Again, the results showed no change in the separation setting or percent recovery. The percent recovery was staying near 40% and the separation setting remained at 1.65 or higher as shown by laboratory float-sink tests.

The next adjustment was to observe the effect of varying the refuse outlet orifice diameter and no change was found.

b. Summary of Results from Adjustment Made on Jigging Cyclones

A summary of the results to improve quality of clean coal recovered produced by the above tests were:

1. Increasing fluid velocity to 17 ft/sec in jigging cyclones did not change the specific gravity separation setting.

2. Changing the percent solids of the slurry feeding the cyclones did not change the specific gravity separation setting, or percent recovery.

3. Variable depth vortex finder settings did not change the percent recovery any noticeable amount, or change the specific gravity separation setting.

4. Different size refuse outlet orifice diameters varied the percent recovery but did not show any specific gravity separation setting change.

OBJECTS OF THE INVENTION

An object of the invention is to provide a method for dimensioning and adjusting at a static position the vortex finder and orifice diameter in a separable shallow dish fitted centrifugal separating cyclone having a single inlet delivering streamlined flow into the centrifugal separating cyclone. A cylindrical bowl having a height comparable to its diameter, a vortex finder set above the top of the dish, an outlet pipe at the top of the cyclone converted to the vortex finder for separation of lights and a single orifice at the bottom of the dish.

A further object of the invention is to provide a wear-resistant centrifugal separating cyclone fitted with separable shallow dish for washing crushed coal having a single inlet with deflector delivering streamlined flow into the bowl as disclosed in my copending application Ser. No. 860,330, filed Dec. 14, 1977, a cylindrical body, a shallow dish, a vortex finder adjusted at the top of the dish for a recovery which depends upon the size, sulfur content, fracturability and ash content of the coal and an orifice diameter which sets the recovery together with the diameter adjustment of the vortex finder.

A further object of the invention is to provide a novel quick replacement type of vortex finder kit for varying the diameter to adjust the recovery of coal as set forth in the preceding paragraph.

A still further object is to provide a new wear-resistant replaceable shallow dish with adjustable surface having critical curvatures, the dish being either of two piece or one piece construction and being insertable at the bottom of the cylindrical section.

A still further object is to provide a set of replaceable wear-resistant orifices of differing diameters for fitting into the dish construction described in the preceding paragraph.

A further object of the invention is to improve the system of coal washing by a new method of combining recoveries of clean coal from high ash and high sulfur

containing coal for meeting the specification for metallurgical grade and steam grade crushed coal by combining relatively low recovery operations in a series of cyclones where the heavies of a first cyclone or series of cyclones at low recovery and relatively high velocity are passed through a second cyclone or second series of cyclones to recover further light fractions therefrom.

A further object of the invention is to provide a system of coal or ore washing by a new method of pulling the light clean coal fraction or ore from the dish and orifice zone at a selected number of revolutions per minute to separate the fraction of clean coal or ore of lower vacuuming resistive forces from the heavier refuse fraction which contains a larger vacuuming resistive force that propels it down and along the curvature of the dish and orifice surface and out through the bottom orifice opening as set forth in the preceding paragraph.

A still further object is to provide a system of coal washing by a new method of recycling the clean coal fraction of a preceding stage through another centrifugal separating stage to expose the clean coal particles with tightly bonded pyrites and other coal impurities to additional centrifugal washing and mixing forces to break these bonds and separate the impurities from the clean coal particles.

A object of the invention is to reduce the wear of the centrifugal involute impeller pump which pumps the pulp slurry to the centrifugal cyclone separator.

A object of the invention is to operate a centrifugal cyclone separator at 8 to 15 psig pressure to reduce wear.

Another object of the invention is to operate a centrifugal cyclone separator with the pulp slurry between 7 and 16 feet per second linear velocity.

A object of the invention is to provide adjustments to the low speed centrifugal cyclone separator in order that light specific gravity particles can be separated from heavy specific gravity particles at different separation ranges e.g. 1.7 sp. gr. range, 1.6 sp. gr. range, 1.5 sp. gr. range, 1.4 sp. gr. range, etc.

Another object of the invention is to feed the inlet pipe to the centrifugal cyclone separator with pre-deflected pulp slurry so as to line the outside wall of the inlet pipe or the wall of the inner separator casing with all or practically all of the solids.

A object of the invention is to manufacture the centrifugal cyclone separator with parts that are replaceable in order that the high wear areas within the separator can be replaced without replacing the entire or practically the entire separator to reduce maintenance and replacement part costs.

SUMMARY OF THE INVENTION

Contrary to the low solids, jigging turbulence and low velocity operations of the prior art, it is a fundamental feature of the present invention and the invention in my Case No. 1, Ser. No. 860,330, that:

(1) the pressure drop between the inlet and the outlet of the cyclone at an operating pump pressure of between 8 and 15 psig be high rather than low, the pressure drop being at least 0.3 atmospheres and preferably up to 1 atmosphere;

(2) the solids content of unwashed coal be at least twice as high, preferably between 2 to 4 times as high (optimally at least 5% and up to 30% solids), compared to that used in Loughner or Visman;

(3) a high flow rate at high solids provide high capacity at lower water requirement for washing than is taught by patents to Vismar or Loughner or in the *Chemical Engineers' Handbook*;

(4) the separating capacity of the shallow bottomed cyclone be increased due to forcing the incoming particles into the cyclone bowl toward the tangential wall by predeflected means;

(5) critical settings of the percent recovery be made of the vortex finder area relative to the bottom orifice area to determine the percent recovery at the top of the cyclone;

(6) the selection of the settings be determined by the amount of ash removal and inorganic sulfur removal from unwashed coal, taking into account the grindability of the coal;

(7) the recovery settings vary from 20% to 70% respectively for efficient washing of 10% to 30% mineral ash coal with the optimum for a clean coal at 8% or below in mineral ash being lower than 70% recovery, 20 preferably 50% to 65%.

(8) the percent recovery setting for washing raw coal having 30% to 40% ash be about 35% to 55% and a single outlet plant with a recycling stage be the only choice for such washing, taking into account the particle size of the coals also affects recovery;

(9) a critical replacable wear-resistant dish geometry and replacable wear-resistant orifice geometry which is unique to the present invention be employed to provide reproducibility of ash removal and inorganic sulfur removal;

(10) the critical geometry of the dish be employed, expressed as the first included angle of entry into the dish,  $\theta_4$ , the second included angle of the dish following the first angle,  $\theta_5$ . Under streamlined flow, the greatest dangers of reentrainment of cleaned coal occurs because of a first turbulence created at the uppermost edge of the dish and thereafter because of a second turbulence created at the lowermost lip of the dish where the whirling vortex enters the orifice structure. This critical first included angle at the entry into the dish,  $\theta_4$ , lies between 80° and 105° and its function is to overcome the turbulence due to abruptly shortening the diameter of the whirling vortex, e.g., compressing the helix. Accordingly,  $\theta_4$  acts as a brake or first gear for the rotational compression of the descending helix. In contrast, Vismar has an equivalent angle corresponding to  $\theta_4$  of 135°.

The second angle,  $\theta_5$ , lies between 100° and 115° for the middle zone which is the 30% to 40% intermediate area of the dish to provide the maximum change in acceleration of the whirling particles in about a 120° sector of one rotation of the helix. If  $\theta_5$  is too high, e.g., about 120° to 125°, the dish is too flat and the necessary separation of clean, light particles does not occur and efficiency drops. The critical rate of downward acceleration represents an increase in velocity which is 2 to 3 times as great in the dish portion as in the cylindrical portion because of the narrow range of  $\theta_5$  between 100° and 115° along a very narrow sector of the revolution. Only  $\frac{1}{2}$  to  $\frac{1}{3}$  of one revolution of the helix is compressed in the dish while the remainder of the revolution is compressed within the orifice structure. Vismar uses the dish portion to create a horizontal partitioning of particles and creates a reverse change from dish to throat curvature lying wholly within the throat of the dish while the change in curvature of the present invention along the common dish orifice wall occurs exclu-

sively in the orifice portion of this common surface. In the invention, the change amounts to about 100°, e.g.,  $\theta_5$  minus  $\theta_9$ , where  $\theta_9$  is the included angle taper in the orifice.

If  $\theta_9$  is substantially less than 12° then the desired throttling compression required in the orifice is not achieved. The last helical revolution of the emerging whirling vortex drops at an accelerated velocity from the top edge of the dish into the central inner portion of the orifice in about the same time along a vertical distance which is 3 times greater than the distance separating adjacent helical turns in the cylindrical portion of the cyclone. This high solids rush towards atmospheric pressure in the constricted orifice creates extraordinary erosion forces.

The invention also is based upon ascertaining the critical setting from analysis of about 190,000 to 200,000 tons of coal the separation characteristics of a shallow bottomed water only cyclone comprising a cylindrical bowl, a single inlet tube, a single bottom orifice in a detachable shallow dish at the cyclone bottom, a fixed vortex finder, a box and an outlet pipe above the vortex finder for removing the light washed particles separated in the cyclone.

A quick-change conical dish supporting plate having openings for nut and bolt fasteners is provided for either a clarifying cyclone, such as the two section long cone dish of Hirsch, U.S. Pat. No. 2,975,896, or for a jiggling cyclone, such as Loughner, U.S. Pat. No. 3,887,456, or for the present squat cyclone of critical height to diameter ratio, preferably 0.90 to 0.95. The quick-change plate permits a change of dish, when worn, change of vortex finder, or change of both, from the bottom.

A new vortex finder sleeve kit is also provided which permits changes to be made for adjusting percent recovery and clean coal quality, e.g., reduction of the mineral ash and inorganic sulfur content. This kit may be installed by tack and stitch welding or, for small diameter cyclones, by mirror welding. A bayonet sleeve kit and cap screws is also described.

The engineering application of critical settings has been summarized in the disclosure of the application for all centrifugal separating cyclones having a broad height to diameter limit of 0.8 to 1.3, preferably 0.90 to 0.95, wherein all cyclone dimensions are expressed in terms of inner bowl diameter, e.g., B. All inlet pipe, outlet pipe, vortex finder sleeve and orifice dimensions are expressed in terms of B and the specific values are shown in Table A herein.

#### BRIEF DESCRIPTION OF THE DRAWING

FIG. 1 is a fragmentary plan view of the centrifugal cyclone of the present invention;

FIG. 2 is a fragmentary elevational view, partly in section, of the cyclone of FIG. 1, having a quick detachable vortex finder sleeve;

FIG. 3 is an enlarged fragmentary vertical sectional view of the cyclone taken on the line 3—3 of FIG. 1;

FIG. 4 is an enlarged fragmentary vertical sectional view through the detachable vortex finder sleeve of the cyclone of FIG. 1;

FIG. 5 is a fragmentary horizontal sectional view, taken on the line 5—5 of FIG. 3;

FIG. 6 is a vertical sectional view, similar to FIG. 3, showing the path of the spiral turns of the processed material within the cyclone as it progresses toward the bottom orifice;

FIGS. 7 and 8 are fragmentary vertical sectional views illustrating modifications of the vortex finder sleeves;

FIGS. 9, 10 and 11 are enlarged vertical, sectional views showing modifications of the cyclone dish and refuse outlet orifice member;

FIG. 12 is a vertical section view of a vortex finder top support plate for giving support to cast vortex finders made of low strength materials.

FIG. 13 is a fragmentary vertical section of a vortex finder made of high wear resistant material e.g. ceramic, cast alloy steels, carbides, etc.

FIG. 14 is a vertical section of a vortex finder sleeve made of high wear resistant material e.g. ceramic, cast alloy steels, carbides, etc.

FIG. 15 is a vertical section of another size vortex finder sleeve made of high wear resistant material e.g. ceramic, cast alloy steels, carbides, etc.

FIG. 16 is a fragmentary vertical section of a centrifugal cyclone separator housing made of a steel outside wall with a high wear resistant inside wall made of ceramic, cast alloy steel, carbides, etc.

FIG. 17 is a fragmentary vertical section of a vortex finder made of off the shelf steel pipe and mechanical tubing with a wear spacer plate shown.

FIG. 18 is a vertical section of a vortex finder sleeve manufactured from steel mechanical tubing.

FIG. 19 is a vertical section of a different size vortex finder sleeve made from steel mechanical tubing.

FIG. 20 is a fragmentary vertical section of a centrifugal cyclone separator housing made of a thin steel outside wall and a replaceable inside wall manufactured from off the shelf steel pipe and mechanical tubing.

FIG. 21 is a fragmentary horizontal view of a right and left hand centrifugal cyclone separators connected to Liller patented streamlining manifold manufactured from Liller patented equalizer T and off the shelf pipe reducers and elbows illustrating path direction of the solids portion of the pulp slurry.

FIG. 22 is a flow diagram of a two stage coal washing plant in accordance with the invention.

FIG. 23 is a graph of the ash removal relative to the percent of recovery;

FIG. 24 is a graph of the inorganic sulphur removal relative to the percent of recovery;

FIG. 25 is a graph of the vortex finder diameter settings, the percent of raw coal ash relative to refuse outlet orifice diameter and the cyclone to percent recovery;

In all of the FIGS. of the drawing, the views are to scale and in accordance with the Examples, which illustrate operations in an 18" cyclone. The representation of the path of the streamlined flow deflected slurry entering the inlet is based upon actual observation and analysis wherein different methods corroborated the particular path which is shown.

The input to each of the cyclone structures is in the form of crushed coal which may vary up to  $1\frac{1}{4} \times 0$  and down to about  $\frac{1}{2} \times 0$ , the range preferred for coal which is difficult to fracture being  $\frac{1}{2} \times 0$  and for easily fracturable coal,  $\frac{1}{2} \times 0$ , other factors, such as high sulfur or ash content, being taken into account. The narrow range of critical settings for dimensions of the structures and parts is summarized, based upon test data, in Table A herein. This Table A expresses all values in terms of B, inner bowl diameter, to permit prediction of other sizes.

## DESCRIPTION OF THE PREFERRED EMBODIMENTS

The embodiments illustrated in the accompanying drawings and following description and examples exemplify the new and patentable changes over my prior application, Ser. No. 860,330, filed Dec. 14, 1977 and show the best modes of carrying out the present invention. These changes comprise:

10 (1) Quick-change mounting plate 32 and fasteners 38 including elongated fixture bolt 38' used for quickly replacing either the vortex finder-sleeve kit 46 or the one piece dish 62, 62A, 72, 82 and 92, orifice 64, 64A, 74, 84 and 94, or both (See FIGS. 2, 3 and 6). Unskilled

15 personnel can change either or both in about five minutes or less. This quick change means is essential in order to quickly accommodate to a different raw coal feed, and to replace the vortex finder-sleeve 46 or to replace a worn dish 62, 62A, 72, 83 and 92, or to install a different size dish 62, 62A, 72, 82 and 92. Any or all of these might have to be done with a change in raw coal and a replacement of a worn part.

(2) Critical Cyclone Dish 62, 62A, 72, 82 and 92 and Vortex Finder Sleeve dimensions 46, 146, 246, 344, 446, and the Empirical Settings shown in FIGS. 23, 24, and 25 and Table A, to maximize clean coal quality and recovery where only the values of raw coal ash, sulfur and fractionability are the variables to determine the required settings of the vortex finder-sleeve.

30 (3) One-Piece Shallow Bottom Dish Orifice 60, 60A, 70, 80 and 90, these best shown in FIGS. 3, 6, 9, 10 and 11 consist of special erosion resistant materials, namely rubber in FIG. 3, alloy in FIG. 6, ceramic liner with rubber layer backing in FIG. 9, ceramic liner with metal backing in FIG. 10, ceramic in FIG. 11, which are suitable materials for all figures.

(4) Quick change Vortex Finder Sleeve Kit shown by elements 46, 146 and 246, is adapted to maximize the quality and recovery of clean coal as shown in FIGS. 40 12, 13, 14, 15, 16, 17, 18, 23, 24, and 25.

(5) Critical Geometry of One-Piece Shallow Bottom Dish-Orifice 60, 60A, 70, 80 and 90, to maximize clean coal quality and recovery as shown in FIGS. 12, 13, 14, 15, 16, 17 and 18.

(6) Operating settings shown in FIG. 25 under (2) to maximize centrifugal separation at selected velocities, raw coal particle size and solids concentration in coal slurry.

(7) Critical location of cyclone parts, shown in FIGS. 50 1, 3, 5, 6, 13, 16, 17, 20, and 21 to minimize wear and avoid turbulence.

### I

55 (1) Quick Change Mounting Plate 32 and Fasteners 38 Including Elongated Pivot Bolt 38'

(a) Relationship of Quick Change Plate Shown In Drawings to Case 1, Ser. No. 860,330, filed Dec. 14, 1977

60 The preferred embodiments illustrated in the drawings are based upon painstaking operations analyses of 200,000 tons of coal washing in the plant and by the method as disclosed and claimed in my prior application, Case No. 1, Ser. No. 860,330, filed Dec. 14, 1977, entitled Inlet Line Deflector and Equalizer Means for a Centrifugal Cyclone Used for Washing and Method of Washing Using Deflectors and Equalizers, and also the divisional applications thereof, namely:

| Case No. | Patent or Serial No. | Issue or Filing Date | Title                                                                                                                                                                                                                                                                                                                             |
|----------|----------------------|----------------------|-----------------------------------------------------------------------------------------------------------------------------------------------------------------------------------------------------------------------------------------------------------------------------------------------------------------------------------|
| I-II     | 4,159,073            | 06/26/79             | Method of Manufacturing<br>Installing an Inlet Line<br>Deflector in a Centrifugal<br>Cyclone for Washing Coal                                                                                                                                                                                                                     |
| I-III    | 4,164,467            | 08/14/79             | Coal Washing Plant Using<br>Deflectors                                                                                                                                                                                                                                                                                            |
| I-IV     | 973,408              | 12/26/78             | Crushed Raw Coal Washing<br>Plant Using A Plurality of<br>Deflector Fitted Centrifugal<br>Cyclones to Produce A Washed,<br>and Dried Mixture of Clean<br>Coarse and Fine Coal, and Fine<br>Coal Alone, with Means to<br>Remove Refuse and Means to<br>Recycle Clean Fine Coal Slurry<br>By-Product into Raw Crushed<br>Coal Inlet |

<sup>(b)</sup>Single and Multi-Stage Operation of the Deflector Fitted Cyclone of Serial No. 860,330, filed December 14, 1977

The centrifugal separation method in my prior application Ser. No. 860,330 had shown tremendous promise when washing George's Creek refuse piles (referred to as Bone Piles). By changing from jig washing to centrifugal washing and adjusting the recovery, FIGS. 23, 24, 25 and 26 the output clean coal quality was improved from 18% mineral ash to 11% mineral ash and a few examples were observed producing 8% mineral ash clean coal.

Applicant's follow-up experiments attempted to discover the 18" cyclone critical settings, FIGS. 23, 24, and 25, Ser. No. 860,330 in a 3-cyclone, 2-stage plant and used run of the mine coal to attempt a vortex setting, FIG. 25 for less than a 1.45 sp. gr. separation. These experiments resulted in a percent of clean coal 30 recovery, FIGS. 23, 24, and 25, for the first stage cyclones 20 of 81.5% average over the first 15 days of operation. However, as the % recovery, FIGS. 23, 24, and 25, of clean coal out the top 24 of the cyclone 20 increased the amount of higher specific gravity particles 40 (refuse) reporting to the clean coal stream also increased throughout the 15 day period. This two-stage, single clean coal outlet, centrifugal cyclone 20 plant, recovered an excessive amount of middlings in the clean coal and failed to produce the desired metallurgical coal 45 quality of less than 8% ash. Although the total 2-stage plant recovery, FIG. 22, using 3 cyclones was correctly set at 75-85% by the vortex finder 146, it was discovered that the percent recovery, FIGS. 23 and 24, was inversely proportional to the clean coal quality, FIGS. 50 23 and 24, and a systematic study was initiated to ascertain the critical settings, FIG. 25, (Ser. No. 860,330).

There is shown in FIGS. 1, 2, 3, 5, 6, 7 and 8 herein a centrifugal cyclone 20 fitted with deflector 23 for creating streamlined flow in a "water only" coal washing. As described in Ser. No. 860,330 and in the divisional applications filed thereunder, the centrifugal cyclone 20 is used to create streamlined flow in a continuous coal washing plant comprising a slurry tank for mixing raw crushed coal and water, a pump feeding the 60 slurry through an inlet 22 into centrifugal cyclones 20, a plurality of centrifugal cyclones 20, each cyclone 20 having two outlets 24 and 26, one outlet 24 at the top and the other refuse outlet 26 at the bottom of each cyclone 20, and one inlet 22 into the cyclone bowl B 65 (28) within housing 27. The inlet 22 is fed by a pump with the slurry of crushed raw coal and water to undergo separation under centrifugal forces whereby

5 clean coal is separated at the top outlet 24 of each cyclone 20 and heavy refuse is withdrawn from the bottom outlet 26. The clean coal consists of coarse coal particles and fine coal particles in water circulating in a closed clean coal circuit as shown in the aforesaid Ser. No. 860,330.

10 It is a critical feature of the aforesaid Ser. No. 860,330 to install a generally flat deflection surface 23 into the inlet tube 22 of each cyclone 20 at three critical angles relative to the inlet tube 22 and cyclone bowl 28:

(1) a center angle made by the inwardly displaced bottom of surface 23 relative to the tube 22 centerline being between 116° and 148°;

15 (2) the deflection angle made by the flat deflection surface 23 relative to the non-tangential feed tube 22 wall being between 8° and 12°; and

(3) the included angle between the radius of the cyclone bowl 28 and the flat deflection surface 23 being between 120° and 170° to thereby separate clean coal at the outlet 24 at the top and refuse at the bottom 26 of the cyclone 20.

20 After separation, the washing process in Ser. No. 860,330 continues by feeding the clean coal output to a dewatering screen to reduce the water content of the clean coal and then to a centrifugal dryer while feeding the separated water containing fine coal below said screen to a fine coal drying circuit.

The method of washing in Ser. No. 860,330 includes feeding the fine clean coal slurry separated in an earlier stage to a clarifying circuit for the removal of the fine clean coal and separating clarified water for reuse in the first, second or third stage slurry tanks in a three-stage process. Each coal batch analysis of sulfur and ash dictated a different optimum dimension of vortex finder diameter D, in order to reach clean coal quality.

The water content of the fine clean coal slurry is reduced by pumping it into clarifying cyclones to separate the slurry into a clarified water portion for reuse in the first, second and third stage slurry tanks and a dewatered portion for further drying to yield a dried clean coal product.

The dewatered fine clean coal with reduced moisture content is produced at a value permitting storage of the centrifugally dried fine coal and the removed fine clean coal particles in water which pass through the fine clean coal centrifugal dryer basket are recycled with the crushed coal in the first, second and third stage slurry tanks with water whereby a constant level of reused fine coal is built up to a value of about 5% in the total plant circuit to push fine clean coal out of the system in continuous operation.

55 FIG. 3 herein shows the separated interior zones 1, 2, 3, 4 and 5 in the cyclone 20 to illustrate vertical layering due to deflector 23. The development of vertical stratification layers 1, 2, 3, 4 and 5 in the cross hatched shading result also from pressure differential between gauges 66 and 68 and the installation of the deflector 23 as is best shown in FIG. 3.

60 Layers 3 and 4 represent the middling coal. In path washing which is the main objective, clean coal transfers into layers 1 and 2, and part of 3 and as illustrated may be the 1.5 specific gravity layer containing the 1.5 specific gravity middlings. Layers 4 and 5 may be the 1.6+ specific gravity layer containing refuse of 2.6+ specific gravity containing clays, pyrites, etc.

65 FIG. 3 herein and FIG. 1 differ in respect to the introduction of threaded pivot or fixture bolt 38' which

is of critical length, threaded at the top and bottom to permit the nut to be shifted from top to bottom, to drop plate 32 while supporting the shallow dish and pivot both dish and plate clockwise for immediate access. The need for the quick opening arrangement also occurs in the frequent requirement to replace parts whose wear alters % recovery and clean coal quality (ash). Recognizing these needs was based upon over a thousand hours of analysis of results of washing and unrecognized mistakes were later uncovered by analyses. Later experiments where the results of FIG. 25 washing in Ser. No. 860,330 show failure to reproduce the limits of washing found in the first experiments, the selected vortex finder settings were found to be altered also by differences in fractionability of the coal, especially in respect to the sulfur content which could be removed by centrifugal washing. Thus, it was obvious that quick changes were needed to make different settings of Vortex Finder D and the detailed aspects are described below.

(c) Distinctive Details of Members 60, 60A, 70, 80 and 90 in FIGS. 3, 6, 9, 10 and 11

It is a critical feature of the present invention shown in FIGS. 3 and 6, that a single circular bottom plate 32, be provided with a single beveled circular central orifice 33, proportioned precisely to encompass the beveled shoulder between the top of the orifice 64, 64A, 74, 84 and 94 and the bottom of the shallow dishes 62, 62A, 72, 82 and 92.

The bottom plate 32 has the appearance of a giant washer and the edges are provided with suitable openings for a plurality of threaded fasteners 38 including elongated fixture bolt 38 of the nut and bolt type. In one embodiment these lie equally spaced on a common circle at the cardinal compass points, for example, 0°, 90°, 180°, 270°. However, two fasteners 38, 180° apart, three fasteners 38, 120° apart, have been used with equal success. Five fasteners 38 are not necessary.

It is a unique advantage of this single circular belt fastened plate 32 with small center hold 33 and fixture bolt 38' that the shallow dishes 62, 62A, 72, 82 and 92, orifices 64, vortex finder housing and vortex finder-sleeve 46 are all fixed by the single plate 32 to share a common axis which is the axis of cyclone 20.

(d) Utility of Quick Change Plate 32 For Jigging Cyclones and Other Cyclones

The novel quick change mounting plate 32 and fastener 38 with elongated pivot bolt 38' is particularly adapted for improving the operation of the jigging cyclone disclosed in Loughner U.S. Pat. No. 3,887,456, and especially for changing the setting of the vortex finder in that patent.

Note that in Loughner, FIG. 1, plate 17 is seemingly fastened to the dish 20 and also is the bottom of the flange 16 at the base of cylindrical bowl wall 11. A plurality of bolts 18 fasten the flange 16 to plate 17 and a plurality of bolts (not numbered) fasten the separable orifice to the bottom portion of the dish 20 and plate. In short, the inner bolts of Loughner connect three parts, e.g., plate, orifice and dish, and the outer bolts connect two parts, plate and the cyclone bottom flange.

Replacing the vortex finder 46, 146 and 246 with another of different diameter requires opening at least two sets of bolts and removing both the dish and orifice together with the bottom plate of Loughner's jigging dish.

Prior to removing the dish, it is required to remove the adhesive cement which bonds dish 20 to the inner bowl wall 11 at 21. Thus, even if a change in vortex diameter dimension is contemplated and dismantling operation is long and complicated regardless of the difficulty of vortex finder replacement and for this reason, this jiggling cyclone cannot be easily adjusted.

In contrast, the invention permits resetting critical parameters determining cyclone operation through the bottom by removing as few as two bolts, partly due to the novel one piece dish-orifice construction and partly due to the novel vortex finder sleeve kit, while uniquely providing a totally new environment for replacement by using an elongated alignment and pivot bolt 38' (FIGS. 2, 3, 6) which can serve as a keeper to hold the one piece dish from the opening in the same flange 16 as in Loughner.

The present invention has attempted to change the vortex finder 46, 146 and 246 diameter by replacement 20 in the apparatus of Loughner first by dismantling the top and then by dismantling the bottom. Dismantling from the top took about one (1) hour. It took about one-quarter (1/4) hour longer to install the new, narrower vortex finder sleeve, and then to fix it.

In contrast, the bottom changing operation in accordance with the present invention takes five (5) minutes or less, using the novel vortex finder sleeve kit 46 of the invention as described in Section (4) below.

Similarly, changing a dish to alter recovery or quality 30 of washed coal in Loughner's jiggling cyclone requires that forty-five (45) minutes to one (1) hour for cement removal and unbolting and rebolting operations. With the invention, the time is about one-tenth (1/10) that in Loughner.

Also, there is no need in the present invention to change the orifice as in Loughner. This need is accomplished in the invention by simply changing the dish 62, 62A, 72, 82 and 92, which with the orifice 64, 64A, 74, 84 and 94, makes one unit 60, 60A, 70, 80 and 90. A new cooperation between dish 62, 62A, 72, 82 and 92 and orifice 64, 64A, 74, 84 and 94 exists in the invention, based upon geometry, Table A, of the one-piece structure 60, 60A, 70, 80 and 90 which is described in Section (5) below.

45 Visman Patent No. RE 26,720 is like Loughner Pat. No. 3,887,456 in respect to requiring opening the cyclone from the top either to change the vortex finder setting, e.g., the distance between the lowest edge of the vortex finder to the top edge of the dish (see FIG. 1 in Visman). In contrast to Loughner's dish which is cemented at the outer thin upper edge to the inner circular wall of the cyclone, Visman bolts his conical dish in the form of a casting as drawn in FIG. 1 by means of bolts through the flange extending outwardly from the top frustum 16 of the cone and this flange of the dish mates with the lower flange of the cyclone bowl.

The present quick change plate fitted with an elongated bolt fixture distinguishes over Visman in permitting immediate access to change the vortex finder from the bottom—there is no corresponding bottom quick change in Visman. Also, there is no need to remove the dish with the quick change plate and fixture bolt when only the vortex finder and its sleeve are changed. The old dish is suspended by means of the fixture bolt. These same differences distinguish over Loughner also.

The vortex finder sleeve it shown best in FIGS. 2, 4, 7 and 8 which is described in greater detail in Part (4) which follows hereafter may be of the weld on type as

shown in FIGS. 7 and 8 or may be of the bayonet socket type shown in FIGS. 2, 4 and 6. To convert from a larger vortex finder area based on the diameter D shown in Table A, to a smaller vortex finder area is the first step needed to reduce recovery of washed coal. This reduction is dictated by the settings illustrated in FIGS. 23 and 24 in meeting the requirements for clean coal quality of metallurgical grade coal as shown in FIG. 22.

A still more important difference over Loughner and Visman, which are the closest prior art to the present invention, is that neither ever conceived the need to change the vortex finder diameter. Only the inventor has made this discovery and it is fully explained in the description of critical parameters which follows.

In summary, the adaptability of the present plate support 32 in combination with the pivoting fixture bolt 38' to every type of cyclone, whether a jiggling cyclone such as Loughner, or a gravity separator as Visman, or pulp clarifier as in Hirsch U.S. Pat. No. 2,975,896 is based upon the discovery that the central aligning opening 33 cooperates with the upper section of the conical dish in each example of these patents to serve as the sole support and to thereby align the center axis of the dish with the center axis of the vortex finder along a common line, the length of the pivoting fixture bolt being just slightly greater than the upper projection dish wall within the cyclone to permit this dish wall to drop a distance which permit pivoting the dish clockwise out of the center of the cyclone to be to a side for while suspended by the fixture bolt.

#### Critical Cyclone Dish and Vortex Finder Dimensions to Maximize Clean Coal

##### A. Parameters Studied

The following parameters were systematically studied: *Structural and Operating Parameters*

1. The correct vortex finder 39 sleeve 46, 146, 246 settings, FIG. 25, were studied to determine the specific gravity separation setting, e.g., the diameter settings;

2. The critical cyclone 20 and cyclone part dimensions, Table A, and settings, FIG. 25, for efficiency limits FIGS. 23 and 24, of centrifugal optimum separation, diameters and heights of cyclone variables;

3. The maximum mineral ash removal, FIG. 23, based on optimum cyclone 20 dimensions, Table A, and settings, FIG. 25, in single and multistage operation

4. The maximum inorganic sulphur removal, FIG. 24, based on the same factors in (3).

5. Washing stage, FIG. 22, required for processing 50 the sizes and different types of raw coal feed.

6. The average particle size of crushed coal before washing.

7. The critical geometry of dish 62, 62A, 72, 83, and 55 92 and bottom orifice 64, 64A, 74, 84 and 94 to maximize the equipment life without reducing separation efficiency, FIGS. 23, 24, and 25 herein cited for efficiencies and FIGS. 3, 6, 9, 10 and 11 herein cited for the dishes.

##### B. Structural and Operational Factors Predetermining Clean Coal Quality

The clean coal quality is controlled by certain factors, some of which are:

1. The percent clean coal recovery setting, FIGS. 23 65 and 24.

2. The inside geometry of the dish and orifice unit 60, 60A, 70, 80 and 90 of FIGS. 3, 6, 9, 10 and 11. Turbu-

lence must be kept at a minimum. Smooth flow is essential. No irregularities can be allowed within the dish orifice unit 60, 60A, 70, 80 and 90 of FIGS. 3, 6, 9, 10 and 11. These set up disturbing flow patterns that cause obvious remixing of clean coal and refuse.

3. The swirling flow stream within the cyclone bowl 27 of FIGS. 1, 2, 3, 5 and 6.

4. The intersection angle in FIG. 5 between the deflector 23 and the tangent of bowl wall 28 of the inlet flow stream developing zones 1, 2, 3, 4 and 5 with the swirling flow stream within the cyclone bowl 28.

5. The depth C of the vortex finder sleeve 46, (Table A) 146 and 246 in FIGS. 2, 3, 6, 7 and 8 between plate 30 and the bottom of vortex finder 46, 146 and 246 of the vortex finder sleeve setting C (Table A) which remain fixed.

6. The height above the inlet 22, called the cyclone bowl head between 22 and 30, which is fixed and kept at zero or a minimum.

7. A smooth gradual transition from the cyclone bowl wall 28 into the dish 62, 62A, 72, 82 and 9 and orifice 64, 64A, 74, 84 and 94 unit 60, 60A, 70, 80 and 90.

8. First conical frustum  $\theta_4$  in dish 62, 62A, 72, 82 and 92. (Table A)

9. Second conical frustum  $\theta_5$  in dish 62, 62A, 72, 82 and 92 and with the combination of (8) and (9) equalling about 100° total included angle from the dish 62, 62A, 72, 82 and 92 entrance to the throat top M.

10. Third conical frustum of continuously changing angle  $\Delta\theta$  from about 110° to about 12° over a short radius section between the dish 62, 62A, 72, 82 and 92 and orifice 64, 64A, 74, 84 and 94 unit 60, 60A, 70, 80 and 90. (Table A)

11. Fourth conical frustum being the included angle  $\theta_9$ , Table A (preferably 12°).

12. Fifth straight cylindrical short sections E and S, Table A.

In items (8) to (12) all conical and tapering sections are adjoined by smooth transition curves so as not to create any abrupt flow disturbances. (See FIGS. 3, 6, 9, 10 and 11 and particularly reference numerals 11 and 12.

13. % Inorganic sulphur removed, FIG. 24 at optimum particle size  $\frac{1}{2} \times 0$  for easily fracturable coal and less for more difficult fracturing coal.

14. The influence of primary mineral impurities in coal on the fracturability in the preparation of  $\frac{1}{2} \times 0$  size crushed coal for washing.

##### C. Critical Factors Effecting Clean Coal Recovery, FIGS. 23, 24, and 25

Clean coal recovery, FIGS. 23, 24, and 25, is controlled by four critical factors of which three are variable and can be adjusted by plant personnel. No. 3 and No. 4 are held constant, leaving only No. 2 for adjustment.

1. The % ash in the raw coal feed to the plant.

2. The diameter D of cylinder 48, 148 and 248 at minimum length of about 0.3B of the clean coal outlet 60 24 called the vortex finder sleeve 46, 146 and 246.

3. The diameter E and length J of the refuse outlet 26 called the bottom orifice 64, 64A, 74, 84 and 94. (Table A)

4. The inside geometry of the dish-orifice unit 60, 60A, 70, 80 and 90 which was solved during the wear problem and it remains fixed.

Although, in the washing of relatively coarse, raw crushed coal in the range of  $\frac{3}{4} \times 0$  to  $\frac{1}{2} \times 0$  and the like, it

has been observed that only about 12% to about 20% of this size crushed coal has a particle size less than 32 mesh to be properly qualified as fines. If the coal is easy to fracture, it has more fines, e.g., closer to 20%.

These fines build up during recirculation of "water only", which is the water medium, and change the recovery settings as shown in FIG. 25. Note clean coal recirculation at the top corners of FIG. 25. This represents a shift in scale to predict cyclone top percent recovery from the vortex finder sleeve diameter.

The percent fines build up can be controlled by the amount of clarifying cyclones 52, shown in FIG. 22. By using more clarifying cyclones 52, the 32 mesh  $\times$  0 fines can be lowered towards the low value of clean coal recirculation shown in FIG. 25, and by using less clarifying cyclones 52, the recirculation of 32 mesh  $\times$  0 fine clean coal approaches the upper value of fine clean coal recirculating.

When the amount of fine clean coal slurry feeding the clarifying cyclone pump 50 approaches the amount of fine clean coal slurry contained in circuits 32 and 46, and with a balanced number of clarifying cyclones 52,

determined by the amount of fine clean coal slurry in circuits 32 and 46 divided by the capacity of the clarifying cyclone 52, the percent recirculation of fine clean coal will be controlled by the efficiency limits of the clarifying cyclone 52 with it approaching the lower value shown in FIG. 25. The amount of unclarified water in circuit 100 in FIG. 22 will approach a minimum value.

When a fewer number than the balanced amount of 10 clarifying cyclones 52 are used, the unclarified water circuit 100 carries 32 mesh  $\times$  0 fines back to the first and second stage slurry tanks 12 and 36, where they begin another trip through the plant circuitry. These fines added to the new fines in the raw coal 10 feed being 15 conveyed into the plant causes a build up of fines and the upper limit of 32 mesh  $\times$  0 clean coal fines recirculating is approached.

It is best for centrifugal cyclone coal washing to use clean water, a balanced amount of clarifying equipment, and keep the amount of fines recirculating at a minimum value.

TABLE A

BEST MODE AND RANGE OF SELECTED CYCLONE DIMENSIONS  
SIZE EXPRESSED IN TERMS OF BOWL DIAMETER AND INCHES  
(ID) OF 18" BOWL SHOWN BY REFERENCE NUMERAL 28 IN  
FIGS. 1, 2, 3, 5 AND 6

| Figure Number    | Reference Number       | Part                                                                | Dimensions of Larger & Smaller Cyclone Parts<br>are Proportional for Each Part to "B" Product<br>Values in Column 6 Below |                          |                         |                     |                 |
|------------------|------------------------|---------------------------------------------------------------------|---------------------------------------------------------------------------------------------------------------------------|--------------------------|-------------------------|---------------------|-----------------|
|                  |                        |                                                                     | Identifying Letter                                                                                                        | Preferred Size in Inches | Expressed in Terms of B | Range in Terms of B | Range in Inches |
| 5,6,7,<br>8      | 28                     | Bowl Diameter                                                       | B                                                                                                                         | 18.0                     | 1.00                    |                     |                 |
| 1,2,3,5<br>6,7,8 | 22                     | Inlet Tube                                                          | A                                                                                                                         | 6.0                      | .33                     | .25-.35             | 4.5-6.4         |
| 3,6<br>6,7,8     | 60 & 48<br>60a & 48    | Vortex Finder<br>Depth Between<br>Vortex Finder                     | C                                                                                                                         | 4.3                      | .23                     | .00-.26             | 0.0-4.8         |
| 3,4,6<br>7,8     | 48,46,<br>148,248      | Vortex Finder<br>Sleeve I.D.                                        | D                                                                                                                         | 6.5                      | .36                     | .30-.50             | 5.5-9.0         |
| 3,6,9,<br>10,11  | 26,75,<br>95           | Orifice Small<br>I.D.                                               | E                                                                                                                         | 3.6                      | .21                     | .16-.25             | 3.0-4.5         |
| 3,5,6            | 44 & 28                | Bowl Width Between<br>$\theta_4$ Included Angle                     | F                                                                                                                         | 4.2                      | .23                     | .20-.31             | 3.6-5.6         |
| 3,6,9<br>10,11   | 60,60a,<br>70,80<br>90 | Depth<br>Dish-Orifice Unit<br>Height                                | G                                                                                                                         | 2.0                      | .11                     | .00-.24             | 0.0-4.4         |
| 3,6,9<br>10,11   | 60,60a,<br>70,80<br>90 | Dish Height, Bet-<br>ween Dish Top &<br>Plate 32                    | H                                                                                                                         | 12.4                     | .69                     | .56-1.0             | 10.0-18.0       |
| 3,6,9<br>10,11   | 60,60a,<br>70,80<br>90 | Height of Orifice,<br>Between Plate 32<br>Top & Orifice Bot-<br>tom | H <sub>1</sub>                                                                                                            | 5.4                      | .30                     | .19-.67             | 3.4-12.1        |
| 2,3,6            | 29 & 32                | Bowl Height Bet-<br>ween                                            | K                                                                                                                         | 22.0                     | 1.22                    | 1.12-1.32           | 20.1-23.8       |
| 3,6              | 30 & 60<br>30 & 60a    | Dish Depth Bet-<br>ween                                             | L                                                                                                                         | 16.7                     | .93                     | .82-1.0             | 14.7-18.0       |
| 3,6,9<br>10,11   | 12                     | Dia. at Throat<br>Entrance to<br>Radius N                           | M                                                                                                                         | 7.1                      | .39                     | .28-.51             | 5.0-9.2         |
| 3,6,9<br>10,11   | 12                     | Radius Connect-<br>ing $\theta_5, \theta_6, \theta_9$               | N                                                                                                                         | 3.5                      | .20                     | .18-.21             | 3.2-3.8         |
| 3,6,9<br>10,11   | 11                     | Radius Connect-<br>ing $\theta_4, \theta_5$                         | P                                                                                                                         | 4.5                      | .25                     | .19-.28             | 3.4-5.1         |
| 3,6,9<br>10,11   | 26,75<br>95            | $\Delta\theta$ Depth or Height<br>of Radius 12                      | Q                                                                                                                         | 2.5                      | .14                     | .06-.28             | 1.0-5.1         |
| 3,6,9<br>10,11   | 64,64a<br>74,84        | Orifice Small I.D.<br>Height                                        | S                                                                                                                         | 1.0                      | .06                     | .00-.22             | 0.0-4.0         |
| 3,6,9<br>10,11   | 64,64a<br>74,84        | Throat Height Bet-<br>ween M & Top of S<br>Orifice Bottom           | T                                                                                                                         | 6.9                      | .38                     | .11-.67             | 1.9-12.1        |
| 3,6,9<br>10,11   | 64,64a<br>74,84        | Outside Dia.                                                        | W                                                                                                                         | 5.0                      | .28                     | .19-.56             | 3.4-10.1        |

TABLE A-continued

BEST MODE AND RANGE OF SELECTED CYCLONE DIMENSIONS  
SIZE EXPRESSED IN TERMS OF BOWL DIAMETER AND INCHES  
(ID) OF 18" BOWL SHOWN BY REFERENCE NUMERAL 28 IN  
FIGS. 1, 2, 3, 5 AND 6

Dimensions of Larger & Smaller Cyclone Parts  
are Proportional for Each Part to "B" Product  
Values in Column 6 Below

| Figure Number | Reference Number | Part                                         | Identifying Letter | Preferred Size           |                         |                          |          |
|---------------|------------------|----------------------------------------------|--------------------|--------------------------|-------------------------|--------------------------|----------|
|               |                  |                                              |                    | Preferred Size in Inches | Expressed in Terms of B | Range in Terms of B      |          |
|               |                  |                                              |                    |                          |                         |                          |          |
| 94            |                  |                                              |                    |                          |                         |                          |          |
| 3,6,9         |                  | $\theta_5$ Depth Between G & M               | Y                  | 2.4                      | .13                     | .00-.33                  | 0.0-6.0  |
| 3,6           |                  | Depth from Inlet 22 to Dish Top 62, etc.     | Z                  | 9.7                      | .54                     | .22-1.0                  | 3.9-18.0 |
| 3,6,9         | $\theta_4$       | Dish Top Included Angle                      | $\theta_4$         | 85°                      |                         | $\pm 15^\circ$           |          |
| 3,6,9         | $\theta_5$       | Dish Bottom Included Angle                   | $\theta_5$         | 110°                     |                         | $\pm 15^\circ$           |          |
| 10,11         | $\theta_6$       | Dish Single Included Angle                   | $\theta_6$         | 100°                     |                         | $\pm 15^\circ$           |          |
| 9,10,11       | $\theta_9$       | Orifice Included Angle Between Radius 12 & E | $\theta_9$         | 12°                      |                         | $+7^\circ$<br>$-3^\circ$ |          |

### E. General Theory of Centrifugal Separation

As stated in Kirk-Othmer *Encyclopedia of Chemical Technology*, Vol. 4, sec. ed. 1964, the capacity of any liquid to solid separation in any centrifugal separator depends upon characteristics of the equipment. This is especially true of cyclones which are adapted to collection and classification of very fine to medium size solid particles in concentrations ranging from very low to medium as well as compressible, gelatinous and amorphous materials that characteristically plug drainage media.

The basic distinction which is presented by the solid treated under gravity centrifugal separation or gravity centrifugal settling is whether the solids are fine or coarse, slow or fast draining. The compactness of all centrifugation equipment lends itself to low or medium tonnages where complete clarity of the liquid effluent is not required. This is ideal for coal washing.

### CENTRIFUGAL SEPARATION

#### (a) Basic Apparatus Postulates for Theory of Operation of the Present Invention

The following are the requirements for the apparatus of the present invention:

1. Crushed coal water is quick draining, noncompressible, nongelatinous, and does not plug draining media.

2. The ash and sulfur impurity has a different specific gravity than the main product and quantity of total ash or sulfur impurity is less than 50% with mineral ash less than 40%, this representing what is defined as a producible coal.

I have discovered that the critical geometry, Table A, of a gravity separating shallow cyclone 20 having a conical bottom with bottom apex angles  $\theta_4$  and  $\theta_5$  of about 85° and 110°, preferably 100° $\pm 5^\circ$  for an equivalent combined angle, is an essential factor which consistently and reproducibly predicts differences of separation, FIGS. 23 and 24, of impurity from the desired product and further predicts the recovery, FIG. 25 or desired product and further predicts the recovery or

capacity FIG. 22 of the cyclone 20 to predetermined the precise adjustments, FIG. 25 of the critical variables of the cyclone 20, which are shown in Table A. The above combined angle  $\theta_4$  and  $\theta_5$  of 100° $\pm 5^\circ$  is  $\theta_6$  in Table A.

#### (b) Function of Cyclone 20 Parts

1. The inlet (22) pipe deflector 23 means creating laminar or streamline flow directs the slurry along the bowl wall 28 of the cyclone 20 in a downwardly tangential helix with all particles layered by gravity from the inside wall 28 outwardly;

2. The vortex finder 44 sleeve 46, 146, 246 area based on the inner diameter D of the cylindrical structure 48, FIG. 4, which functions to withdraw lights above the shallow bottom 60, 60A, 70, 80 and 90;

3. The outlet orifice 64, 64A, 74, 84 and 94 diameter E which functions as a partial baffle or restrictor in its critical relation to the vortex finder 44 sleeve 46, 146, 246 area sizing to expand or to compress the number of helical turns, see FIG. 6, 170, in the tangentially streamline laminar flow and to further effect a smooth streamlined layered outflow of layered product through the vortex finder outlet pipe 44 above the vortex finder sleeve 46, 146, 246 from the bottom separation zone within the dish-orifice 60, 60A, 70, 80 and 90;

4. The spacing C of the vortex finder 44 sleeve 46, 146, 246 permits the smooth withdrawal of upward flow so that through the vortex finder 44 from the super gravity zone in the bottom cone 60, 60A, 70, 80 and 90, must be no more than 90% of the straight side wall height L of the cyclone 20 measured from the top edge of the cone 60, 60A, 70, 80 and 90 to the top 30 along inner wall 28 of the cyclone 20;

5. Pressure differential of at least 0.9 up to 1.8 preferably 1.5 $\pm 0.2$  atmospheres between the inlet tube 22 and the outlet pipe or vortex finder 44, the latter both being at atmospheric pressure thereby fixing the initial super gravity forces which maintain the essential separation between the vertical layers 1, 2, 3, 4 and 5 in FIGS. 3 and 5 in the straight side wall 28 section of the cyclone 20 and which maintain the high velocity momentum of

the heavy particles in the conical bottom 60, 60A, 70, 80 and 90 departing from the restricted bottom orifice 64, 64A, 74, 84 and 94 to prevent undesired contamination of the light particles removed through the vortex finder 44. The high velocity momentum based on gravity, and the centrifugal velocity in the cyclone 20 and the abrupt change in direction at the bottom cone in 60, 60A, 70, 80 and 90 is sufficient under a  $\Delta p$  of 1.5 atmospheres to completely overcome a tendency to wander from the outer conical wall in 60, 60A, 70, 80 and 90 zone 10 towards the vacuuming zone within the vortex finder 44. See FIG. 3 for estimating short critical lateral cross-over distances.

#### (c) Preserving Streamline Flow

For sharp separation of different specific gravity materials in cyclone 20 apparatus a smooth streamline flow must be created at the entrance 22 when the material first enters the cyclone bowl 28; in order that smooth layers 1, 2, 3, 4 and 5 of different specific gravity particles will be created and aligned. The different specific gravity materials must be allowed to seek their respective layers 1, 2, 3, 4, and 5. Refer to Case No. 1, Ser. No. 860,330, for creating the layers 1, 2, 3, 4 and 5.

It is very critical that these layers 1, 2, 3, 4 and 5 are not destroyed until each one has departed from the cyclone bowl 28 and bottom unit 60, 60A, 70, 80 and 90. Prior art focused on separation within the bowl without considering the development of the reverse flow path and the effect this development had on each of the 30 different specific gravity layers 1, 2, 3, 4 and 5 and the circular helical fluid velocity of 15 to 28 feet per second in the separating zone in 60, 60A, 70, 80 and 90 at the bottom conical portion of the cyclone bowl 28.

The laminar streamline flow develops two desirable 35 situations.

The first creation of different specific gravity solid material layers 1, 2, 3, 4 and 5 lines up the materials swirling around the upper portion of the cyclone bowl 28 with the heaviest materials against the bowl wall 28 40 and the corresponding layers containing lighter materials as you travel away from the bowl wall 28 towards the vortex finder 44 wall. This alignment of materials sets the stage for the vacuuming operation. It is very critical that the solid particle helical 170 circular velocities be maintained while the particles are in the cyclone bowl 28 thus the reason for the squat cyclone to permit about 2 to 3 turns before entering the dish 62, 62A, 72, 82 and 92 zone. Once the light particles enter the vortex finder 44 sleeve 46, 146, 246 inner diameter D or the 45 heavy particles enter the bottom orifice 64, 64A, 74, 84 and 94 inner diameter E, the helical 170 circular fluid velocities are no longer critical. Velocity may be radians per second (RadPS), rpm or Rp.

The quantity of material (pump slurry) being pumped 55 for an 18" classifying cyclone 20 of my co-pending patent application Ser. No. 860,330 should be about 1500 GPM of 10 to 35% solid slurry. This flow quantity will yield the necessary entrance fluid velocity of from 15 to 28 feet per second for cyclones 20 equipped with 60 the streamline flow deflector 23 to provide the centrifugal forces necessary in the dish 62, 62A, 72, 82 and 92 and orifice 64, 64A, 74, 84 and 94 separation zone within 60, 60A, 70, 80 and 90. See FIG. 3 for separation.

#### (d) Vacuuming Forces

The vacuuming forces are developed by the pressure differential between the inlet pipe 22 and the vortex

finder 44 sleeve 46, 146, 246 inner diameter D outlet 24. The pressure differential must be in the order of 0.9 to 1.8 atmospheres to develop the vacuuming forces necessary to separate more efficiently the solid particle layers 5 1, 2, 3, 4 and 5 as they enter the separation zone within 60, 60A, 70, 80 and 90. The stage is now set for selective separation by particle specific gravity and not by particle size.

All particles must have enough helical circular 170 velocity momentum in order that the higher specific gravity particles will have enough centrifugal force at the correct RPM within 60, 60A, 70, 80 and 90 to overcome the vacuuming force in the separation zone within 60, 60A, 70, 80 and 90 and maintain their position in the

15 outer heaviest particle layers 4 and 5 and report to the bottom orifice 64, 64A, 74, 84 and 94 outlet 26 and out of the cyclone 20. If the solid particles had not been layered according to particle specific gravity, it is possible for some of the heavier specific gravity particles to be vacuumed away up through outlet 24 with a large amount of the light specific gravity particles thus misplacing material, which does occur after considerable use of the cyclone 20 due to flow disturbances created by wear.

The amount of vacuuming desired depends on the percentage of recoverable light specific gravity particles being processed and the RadPS. desired in the vacuuming zone within 60, 60A, 70, 80 and 90 which determines the specific gravity separation setting. The larger the percentage of recoverable light specific gravity particles, the larger the vacuuming area necessary to recover the particles. Vice versa for the smaller the percentage of recoverable light specific gravity particles, the smaller the vacuuming area. The vacuuming area is controlled by the inner diameter D and the length of about 0.3B minimum of the vortex finder 44 sleeve 46, 146, 246.

#### (e) Pressure Differential For Vacuuming Forces

The test runs using both laminar streamline flow and nonlaminar flow at flow rates between 800 and 1500 GPM produced a large difference of 7 psi in pressure differentials between inlet 22 and outlet 24 and a large observable circular helical 170 swirling fluid velocity difference. The pressure differential of 0.9 to 1.8 atmospheres was produced only when laminar streamline flow was used. The maximum pressure differential obtained without laminar streamline flow was 8 to 13 psi gauge. Very poor separation of low and high specific gravity particles was observed.

The poor separation without streamline flow was blamed more on not forming the different smooth layers 1, 2, 3, 4 and 5 than on the lower pressure differential. But it is obvious that when the centrifugal force of the particles is increased by the high circular helical 170 fluid velocities (15 to 28 feet per second) that a greater pressure differential will be required to vacuum the low specific gravity particles off the high specific gravity particles.

As the particles under angular acceleration with increasing angular velocity enter the separation zone within 60, 60A, 70, 80 and 90, the different specific gravity materials will have a wider range of vacuum resistance forces thus making the light specific gravity 65 particles easy to vacuum compared to the higher specific gravity particles which are very difficult to vacuum at these centrifugal forces created by helical 170 swirling linear fluid velocities between 15 and 28 feet

per second at the separation Rad PS required within 60, 60A, 70, 80 and 90. See FIG. 6 for angular acceleration in terms of Rad PS.

At low circular helical 170 fluid velocities in the separation zone at the bottom conical portion within 60, 60A, 70, 80 and 90 of the cyclone 20, the vacuuming resistance forces of the light and heavy specific gravity particles have a much closer value thus both types of particles being predominant. This causes misplaced material and a low quality clean coal product. Also, some of the larger light specific gravity particles report to the bottom orifice 64, 64A, 74, 84 and 94 outlet 26 proven by refuse washability tests.

(f) Effect of Compression Before and Loss of Compression After

The large observable circular helical 170 swirling fluid velocity difference was observed by the physical characteristics of the plant operating. With the nonlaminar flow a large amount of noise and plant vibrations were present. The cyclones themselves shook from flow resistance. When the flow was changed to laminar streamline flow, the speed of the material was such that the same bottom orifice used with the nonlaminar flow, producing 70% plant recovery for a two-stage circuit allowed about all of the raw coal to be discharged out through the bottom orifice. The bottom orifice was changed from a 0.236B" I.D. to a 0.208B" I.D. to yield the same 70% plant recovery. Obviously, the velocity through the cyclone was increased very significantly when using laminar streamline flow to empty the cyclone bowl 28 so fast when using the exact same bottom orifice. All noise and vibrations stopped when laminar streamline flow was used. The surprising discovery was that clean coal ash dropped from 18%-20% in turbulent flow down to 8-11% in streamline flow.

(g) Basic Theory Differences Between Centrifugal Separation and Jigging Separation

| Jigging Cyclone                                                                                                                         | Centrifugal Separation Cyclone 20                                                                                                                               |
|-----------------------------------------------------------------------------------------------------------------------------------------|-----------------------------------------------------------------------------------------------------------------------------------------------------------------|
| (a) Low Velocity                                                                                                                        | (a) High Velocity                                                                                                                                               |
| (b) High Kinetic Energy Due to Turbulence                                                                                               | (b) Substantially Zero Kinetic Energy Due to No Turbulence                                                                                                      |
| (c) Low Potential Energy Due to Low Velocity and Low Pressure Differential as Indicated by Inlet Pipe Gauge 66 and Outlet Pipe Gauge 68 | (c) High Potential Energy Due to Pressure Differential Between Inlet 22 Pipe Gauge 66 and Light Fraction Outlet 24 Pipe Gauge 68 Which is .9 to 1.8 Atmospheres |
| (d) Very Low Super Gravity (.5 to 0.8 atmospheres)                                                                                      | (d) High Super Gravity Forces (.9 to 1.8 atmospheres)                                                                                                           |

Centrifugal Separation At Low PSIG, Velocity, And Wear

Pumping high coal solids slurry e.g. 5 to 30% solids with slurry pumps e.g. centrifugal impeller type causes severe wear to the casings, housings, and the moving parts which the slurry contacts. The faster the pump is operated the more severe the wear and the slower the pump is operated the less severe the wear.

It has been found that the centrifugal cyclone separator 320 and 420 of FIG. 21 can be operated between 8 and 18 psig pressure with a pressure differential between 0.3 and 1.0 atmospheres, at 7 to 17 feet per second

slurry velocities and produce separation ranges between 1.4 and 1.7 specific gravity.

Manifold Deflection

5 The discovery was made when the manifold 389 shown in FIG. 21 was coupled with a right hand inlet separator 320 and a left hand inlet separator 420.

10 The manifold 389 precisely divides the pulp slurry into two equal proportions by use of the flow equalizer T 387. The two equally divided streams are then deflected at each end of the manifold by the end elbows 377. This sudden turn by the pulp slurry streams forces the particles of the stream by centrifugal force to seek the outside wall of the inlet feed pipe 322 and 422 to the centrifugal cyclone separators 320 and 420 and streamline the flow.

15 This deflection of the pulp slurry stream produced a new set of specific gravity separation ranges for the tangentially fed centrifugal cyclone separators 320 and 420 shown in FIGS. 23, 24, and 25.

Bowl Wall Wear And Wear Resistant Materials

The placement of practically all of the solids on the centrifugal cyclone separator bowl wall 28 in FIGS. 3, 5, and 6 increases the severity of the wear to the wall. To reduce the maintenance and replacement cost when repairing the worn out wall 28 a replaceable bowl wall liner 351 and 451 made of either steel, hard metal alloys, urethane, tungsten molybdenum carbide alloy, chromium carbide alloy, tungsten-chromium titanium carbide alloy are used. The foregoing alloys may be modified with cobalt.

Hard Alloy Materials For Bowl Liner 451

Another preferred wear resistant alloy is a mixture of 5% fine grain tungsten carbide and 95% coarse grain tungsten carbide alloy which is stabilized with a small amount (0.1 to 0.2) of vanadium carbide and hardened with about 0.2% chromium. Another preferred alloy is 40 the foregoing tungsten carbide alloy with vanadium carbide alloy to which is added about 6 to 15% of cobalt for increased ductility. Fabrication of this alloy is made in accordance with the specifications given in the Handbook of Hard Metals by W. Dawihl, copyrighted 1955 by Her Majesties Printing Office in Great Britain.

Ceramic Composition Of Bowl Liner 451 In FIG. 16

50 A magnesia spinel (formula  $MgAl_2O_4$ ) is a preferred ceramic which can be made by the technique as used in manufacturing the lining for a molten steel crucible by using a parting agent and making a slip in a mold (plaster of Paris) in the shape of the liner 351 and 451. The liner must be fired at high temperatures to convert it to magnesia spinel.

Another ceramic which can be used is a cast and fired ball mill lining composition based on aluminum for the liner 451 in FIG. 16. The  $Al_2O_3$  composition of British Pat. No. 454,946 of Apr. 4, 1935 is made as shown in these patents. Another unit 451, FIG. 16 is made of at least 97% pure  $Al_2O_3$  composition.

Steel Bowl Liner 351 In FIG. 20

A steel liner for an 18" separator made from off the shelf available steel pipe shown in Marmon/Keystone Corp. 1979 Stock List can be cost effective. For example by making the centrifugal cyclone separator casing 355 with off the shelf pipe size 20" O.D./in.  $\times$  0.438" Wall/in. or size 20" O.D./in.  $\times$  0.375" Wall/in., the

separator bowl liner 351 can be made with 19" O.D./in.  $\times$  0.750" Wall/in. or 19" O.D./in.  $\times$  0.500" Wall/in. providing a replaceable wall without the need to remanufacture the entire separator 320.

The dish and orifice unit 90 housing 357 and 457 shown in FIGS. 16 and 20 can be made similarly to facilitate the replacement of the bowl liners 351 and 451.

#### Combined One Piece Separator Casing And Lining

The 18" centrifugal cyclone separator bowl housing 27 shown in FIG. 2 and 6 can be made from off the shelf steel pipe as shown in the 1979 Stock List with a one piece 20" O.D./in.  $\times$  0.812" Wall/in. or 20" O.D./in.  $\times$  1.031" Wall/in. when the wear becomes severe enough to impair the separator 20 performance.

#### Replaceable Vortex Finder Sleeve Adjustment

Another severe wear area of the centrifugal cyclone separator is in the vortex finder inside surfaces as shown in FIGS. 3, 4, 6, 7, 8, 13, 14, 15, 17, 18, and 19. A one piece vortex finder outlet tube as shown in FIGS. 2, 3, 4, 6, 7, 8, and 13 can be used, but due to the severity of the wear within the inside surfaces due to corrosion and erosion only the one piece outlet tube 444 when made from highly wear and corrosion resistant materials listed under Hard Alloy and Ceramic Materials For Bowl Liner 451 can withstand the abrasive forces for long periods of time.

#### Steel Pipe And Mechanical Tubing Vortex Finders

Steel vortex finders made from off the shelf steel pipe and mechanical tubing as shown in FIGS. 17, 18, 19, and 21 are cost effective. The top outlet pipe 339 is made from 8" sch. 40 pipe. The vortex finder annular fix space pipe 341 is made from standard, off the shelf steel pipe as shown in the Marmon/Keystone Corp. 1979 Stock List, size 9 $\frac{1}{2}$ " O.D./in.  $\times$  0.375" Wall/in. The top V.F. cover plate 329 is made with at least  $\frac{1}{8}$ " steel plate.

The three parts 339, 341, and 329 are welded together as shown in FIG. 17 by welds 335. The wear spacer ring 330 can be made from steel or other cost effective wear resistant materials as previously mentioned. If no wear spacer ring 330 is used then a thicker top plate 329 is required to give a longer wearing life to the cyclone top.

As previously mentioned the inside surfaces of the vortex finder 39, 139, 239, etc. and the sleeve kit as shown in FIGS. 2, 3, 4, 6, 7, 8, 13, 14, 15, 17, 18, and 19, all experience severe wear. By manufacturing the sleeves 446, 447, and 448 from ceramic and other highly corrosion and abrasion resistant materials increased life can be obtained, but added mold expenses and manufacturing costs makes the all steel sleeves 46, 146, 246, 343, 344, and 345 more attractive, even though they must be changed more frequently; because they can be made from off the shelf steel mechanical tubing as shown in Marmon/Keystone Corp., 1979 Stock List for pipe and mechanical tubing.

By using a vortex finder interior wear sleeve 337 held in place by the sleeve flange 350 as shown in FIG. 17, the short wear life of steel can be tolerated due to the ease and expense of changing a worn out sleeve with a new insertable sleeve 337.

#### Centrifugal Cyclone Separator Operational Ranges

A right and left hand non-deflector inlet centrifugal cyclone separator as shown in FIG. 21 has an operating pressure range of 8 to 18 psig at the manifold pressure

gauge 488. A 5 to 40% solids slurry fed to the streamlined manifold 389 at 6 to 16 feet per second velocity gives the energy requirement for centrifugal separation with minimum turbulence. The arrows in FIG. 21 show the path of travel of the solids material as it passes through the equalizing manifold and into the top of the centrifugal cyclone separators 320 and 420.

At the upper limit of 18 psig pressure, turbulence increases due to the high velocity mushrooming in the entrance at the top of the cyclone annular section.

The streamlined manifold 389 consists of a equalizing T 387 as taught in Liller patent application Ser. No. 860,330, two pipe reducers 378 to minimize loss of pumping energy and velocity, two elbows for deflecting the flow at the ends of the distributor line towards the outer surfaces of the outlet pipes 379 leading into the cyclone bowls 355 and 455, and the pressure gauge 488 for reading operating conditions.

#### Deflected Inlet Centrifugal Cyclone Separator

The deflected inlet centrifugal cyclone separator as described in my co-pending patent application Ser. No. 860,330 has an operating pressure range of 8 to 35 psig at 6 to 35 fps velocities by limiting the inlet restriction to about 33%. Restricting the centrifugal cyclone separator inlet 22 by 35% and more increases the inlet fluid velocity by large factors creating violent turbulence due to a high velocity stream (inlet fluid velocity) intersecting a low velocity stream (annular fluid velocity).

For example:

a 35% reduction in the cyclone bowl inlet increases the cyclone bowl inlet fluid velocity by 53.85%;

a 50% reduction in the cyclone bowl inlet increases the cyclone bowl inlet fluid velocity by 100%;

a 70 and 85% area reduction increases the cyclone bowl inlet fluid velocity by 233.35% and 566.65% respectively. The solution to the violent turbulence was the critical geometry deflector reducing the inlet pipe area by about 19 to 32%.

TABLE

INLET PIPE, CYCLONE INLET, AND ANNULUS FLUID VELOCITIES, AREA  
VERSUS PERCENT CYCLONE INLET/REDUCTION FOR  
AN 18" CENTRIFUGAL CYCLONE SEPARATOR

Inlet pipe area = 28.27 in<sup>2</sup> = 0.1963 ft<sup>2</sup>

| Cyclone<br>Feed<br>Inlet Pipe<br>Fluid<br>Velocity<br>in FPS | %<br>Cyclone<br>Inlet<br>Area<br>Reduction | Cyclone<br>Bowl<br>Inlet<br>Fluid<br>Velocity<br>in FPS | Annulus<br>Fluid<br>Velocity<br>at inside<br>bowl wall<br>in FPS | % Increase in<br>Cyclone Bowl<br>Inlet Fluid<br>Velocity<br>over the<br>Inlet Pipe and<br>Annulus Fluid<br>Velocities |
|--------------------------------------------------------------|--------------------------------------------|---------------------------------------------------------|------------------------------------------------------------------|-----------------------------------------------------------------------------------------------------------------------|
| 20                                                           | 0.00                                       | 20.00                                                   | 20                                                               | 0.00                                                                                                                  |
| "                                                            | 5.00                                       | 21.05                                                   | "                                                                | 5.25                                                                                                                  |
| "                                                            | 10.00                                      | 22.22                                                   | "                                                                | 11.10                                                                                                                 |
| "                                                            | 15.00                                      | 23.53                                                   | "                                                                | 17.65                                                                                                                 |
| "                                                            | 20.00                                      | 25.00                                                   | "                                                                | 25.00                                                                                                                 |
| "                                                            | 25.00                                      | 26.67                                                   | "                                                                | 33.35                                                                                                                 |
| "                                                            | 30.00                                      | 28.57                                                   | "                                                                | 42.85                                                                                                                 |
| "                                                            | 35.00                                      | 30.77                                                   | "                                                                | 53.85                                                                                                                 |
| "                                                            | 40.00                                      | 33.33                                                   | "                                                                | 66.65                                                                                                                 |
| "                                                            | 45.00                                      | 36.36                                                   | "                                                                | 81.80                                                                                                                 |
| "                                                            | 50.00                                      | 40.00                                                   | "                                                                | 100.00                                                                                                                |
| "                                                            | 55.00                                      | 44.44                                                   | "                                                                | 122.20                                                                                                                |
| "                                                            | 60.00                                      | 50.00                                                   | "                                                                | 150.00                                                                                                                |
| "                                                            | 65.00                                      | 57.14                                                   | "                                                                | 185.70                                                                                                                |
| "                                                            | 70.00                                      | 66.67                                                   | "                                                                | 233.35                                                                                                                |
| "                                                            | 75.00                                      | 80.00                                                   | "                                                                | 300.00                                                                                                                |
| "                                                            | 80.00                                      | 100.00                                                  | "                                                                | 400.00                                                                                                                |
| "                                                            | 85.00                                      | 133.33                                                  | "                                                                | 566.65                                                                                                                |

The specific gravity separation range settings of the deflected and non-deflected inlet centrifugal cyclone separators operated in accordance with the present invention are as follows:

| Specific Gravity Separation Range | Inside Diameter Area Of Vortex Finder Sleeve 46, 146, 246, 343, 344, 345, 446, 447, or 448 In Square Inches For A Centrifugal Cyclone Separator With |                                  |
|-----------------------------------|------------------------------------------------------------------------------------------------------------------------------------------------------|----------------------------------|
|                                   | Deflected Inlet S.N. 860,330 8 to 35 psig                                                                                                            | Non-Deflected Inlet 8 to 18 psig |
| 1.65                              |                                                                                                                                                      | 50                               |
| 1.60                              |                                                                                                                                                      | 48                               |
| 1.55                              | 55                                                                                                                                                   | 41                               |
| 1.50                              | 48                                                                                                                                                   | 33                               |
| 1.45                              | 41                                                                                                                                                   | 25                               |
| 1.40                              | 33                                                                                                                                                   |                                  |
| 1.35                              | 25                                                                                                                                                   |                                  |

The largest centrifugal cyclone separator inlet restriction of about 33% coupled with the largest deflection angle of about 13° permits going to the highest velocities. As the velocities are reduced so can be the restriction and deflection angle.

### III.

#### One Piece Shallow Bottom Dish-Orifice Unit of Erosion Resistant Material

##### A. Introduction

Although all cyclones are fitted with an orifice at the dish bottom whose diameter can be related to the cyclone bowl diameter, relatively few prior patents in the art of centrifugal separation teach replacement of the orifice element or teach an optimum relationship based upon added factors of clean coal quality and % recovery. Only Loughner, already mentioned, suggested changing the diameter but gave no advise on what values produce desired results.

Hirsch U.S. Pat. Nos. 2,975,896 and Fitch, Jr. et al. 3,501,014 mention desirable values of outlet orifice diameter which can be related to cyclone bowl diameter but Hirsch teaches a very long cone totally different from that of the inventor while Fitch, Jr. et al. mentions varying such parameters as bowl diameter, orifice diameter, inlet diameter and vortex finder diameter.

To facilitate understanding the invention with respect to the closest prior teachings in Fitch, Jr. et al. the comparison is made below:

| Fitch, Jr., et al.                                                                                               |               | The Present Invention                                                                             |      |
|------------------------------------------------------------------------------------------------------------------|---------------|---------------------------------------------------------------------------------------------------|------|
| Regenerative Cyclone Operating Under Increased Residence time and Reduced Velocity in cone to Reduce Drag forces |               | Decreased residence time with Increased radial velocity in Conical portion. Increased drag forces |      |
| Inlet capacity                                                                                                   |               | Inlet capacity                                                                                    |      |
| Cyclone 200 GPM                                                                                                  |               | Cyclone 900 GPM                                                                                   |      |
| Col. 6, lines 10-18 particularly line 11                                                                         |               | Liller velocity six times greater than Fitch                                                      |      |
| Higher inlet velocities                                                                                          |               |                                                                                                   |      |
| Relationship of Orifice to V.F. Diameter in 12" Cyclone                                                          |               |                                                                                                   |      |
| In Terms of B                                                                                                    | Ratio Do/Du   | Ratio Do/Du                                                                                       |      |
| .25 Do = 3"                                                                                                      | .36 Do = 4.32 |                                                                                                   |      |
| .08 Du = 1"                                                                                                      | 3             | .21 Du = 2.40                                                                                     | 1.75 |
| Do-Du = 2                                                                                                        |               | Do-Du = 1.82                                                                                      |      |

The most severe wear occurs in the throat Q of the orifice 62, 62A, 72, 82 and 92 and tapers out in both

directions. For this reason the dish 64, 64A, 74, 84 and 94 and orifice 64, 64A, 74, 84 and 94 should not be separate parts. The separate dish 62, 62A, 72, 82 and 92 and orifice 64, 64A, 74, 84 and 94 metal parts showed severe wear at the mating surface. An orifice 64, 64A, 74, 84 and 94 and dish 62, 62A, 72, 82 and 92 designed and molded as one unit 60, 60a, 70, 80 and 90 is best.

A cast steel alloy known as "Ni Hard" forms the dish and orifice unit 60A in FIG. 6. The castings wore out after 3000 tons of coal processed. This casting contained 18% Cr, 8% Ni, up to 25% Cr and 12% Ni

During the trial and error periods of production of about 100,000 tons changes in materials shown in FIGS. 3, 6, 9, 10, and 11 were tested and observations made with the object of reducing the wear pattern to produce an optimum design for reproducibility and increasing the quality of the coal being produced.

When the dish was made of Adiprene (FIG. 3) the single unit dish 60, and the orifice part 64 lasted about 5000 tons with no change in separation efficiency, e.g. with good reproducibility throughout its life.

The wear occurs evenly and smoothly and no gouging is observed causing flow irregularities. The curvature geometry remains constant. All radii from the bottom section at (65, 65A, 75, 85, and 95) of the orifice 64, 64A, 74, 84 and 94 (See FIGS. 3, 6, 9, 10 and 11) to the top M of the throat radius 12 change at a uniform rate thus maintaining the  $\theta_9$  included angle and also maintaining about the 0.19B inch radius e.g., radius 12 from the  $\theta_9$  included angle to the top M of the throat; this insures that there will be no change in coal quality as the orifice 64, 64A, 74, 84 and 94 sleeves wear out.

##### (C) Change in Percent Recovery During Wear:

The greatest change in recovery, as predicted by the Cyclone Recovery Graph in FIG. 25, illustrates the effects of the diameter of vortex finder sleeve 46, 146, 246, size D, and orifice 64, 64A, 74, 84, 94, diameter E, in Table A versus cyclone top percent recovery (see FIGS. 23, 24 and 25) occurring between 0.20B and 0.23B the range of orifice diameter E. Between 0.20B and 0.22B of wear, the difference in wear represents  $\frac{2}{3}$  of 0.03B, which is  $\frac{2}{3} \times \frac{1}{2}$ , or  $\frac{1}{3}$  of wear in an 18" cyclone. As shown in FIG. 25, a decrease in wear of  $\frac{1}{3}$  results in about 6% change in recovery, e.g., a decrease which is surprisingly low. It was also discovered that wear between 0.22B and 0.23B, e.g., the last 2/9 of the wear, causes an 11% to 12% loss of recovery, shown in FIG. 25.

These surprising discoveries established that the orifice geometry (64, 64A, 74, 84 and 94) can be allowed to wear in a significant manner to approximately the 0.22B diameter value, e.g., the value of E can change to a certain degree without substantially changing the plant percent of recovery. The cyclone plant used an Adiprene dish 62 and bottom orifice 64 in the total Adiprene unit 60, FIG. 3. A similar result of only 5% to 6% loss of recovery, when using other wear resistant materials with geometry monitored in precisely the same manner, was discerned.

##### (D) Wear Test Results for Adiprene Rubber Units 60 in FIG. 3.

The different dish 62 and orifice 64 materials tested indicated that the Dupont Adiprene (polyether urethane L-100) 83 to 85 Durometer, Shore A, 60, FIG. 3,

is the best rubber material. The following table shows typical test results.

TABLE B

| Rubber and Shore A Hardness                                    | Number of Eight Hour Shifts of Satisfactory Wear |
|----------------------------------------------------------------|--------------------------------------------------|
| 1. Polyether Urethane Dupont Adiprene L-100 83 to 85 Durometer | 10                                               |
| 2. Polyester Urethane 90 Durometer                             | 3                                                |
| 3. Polyester Urethane 80 D                                     | 8                                                |
| 4. Polyether Urethane 90 D, 95 D Dupont Adiprene L-100         | 1                                                |

In Table B increasing the hardness of the urethane rubber reduces the wear resistance. The best hardness is 83 to 85.

Lowering the hardness to about 70 Durometer Shore A is totally unsatisfactory and causes both a loss of tear strength and of toughness.

Applicant has also found that American Cyanimide Co. produces a urethane material similar to Dupont's Adiprene which wears as well as the Trial No. 1.

(E) Hard Alloy Materials for Dish 62A and Orifice 64A

The preferred non-rubber material for the dish 62A and orifice 64A is a hard metal alloy such as tungsten molybdenum carbide alloy, chromium carbide alloy or a tungsten-chromium titanium carbide alloy. The foregoing alloys may be modified with cobalt. An outer holder of steel 80, FIG. 10 and a liner 86, FIG. 10.

Another preferred wear resistant alloy is a mixture of 5% fine grain tungsten carbide and 95% coarse grain tungsten carbide alloy which is stabilized with a small amount (0.1 to 0.2) of vanadium carbide and hardened with about 0.2% chromium. This is the preferred wear resistant alloy used in FIGS. 6 and 10 for parts 60A and 80. Another preferred alloy is the foregoing tungsten carbide alloy with vanadium carbide alloy to which is added about 6% to 15% of cobalt for increased ductility. Fabrication of this alloy is made in accordance with specifications given in the Handbook of Hard Metals by W. Dawihl, copyrighted 1955 by Her Majesties Printing Office in Great Britain.

Ceramics as set out in Section (F) below can also be used as the wear resistant material for 70, 80 and 90 in FIG. 9, 10 and 11.

(F) Ceramic Composition of Dish in FIGS. 9, 10 and 11

A magnesia spinel (formula  $MgAl_2O_4$ ) is a preferred ceramic which can be made by the technique as used in manufacturing the lining for a molten steel crucible by using a parting agent and making a slip in a mold (plaster of Paris) in the shape of the liner 76 and 86. The dish must be fired at high temperatures to convert it to magnesia spinel.

Another ceramic which can be used in a cast and fired ball mill lining composition based on aluminum for the dish and orifice units 70 and 80, FIG. 9 and 10. The  $Al_2O_3$  composition of British Patent No. 454,946 of Apr. 4, 1935 is made as shown in these patents. Another unit 90, FIG. 11, made entirely of  $Al_2O_3$  composition is also used.

(G) Effect of % Solids, Particle Size, Fracturability, Raw Coal Feed Velocity, Mineral Ash Content and Inorganic Sulfur Content on the Wear of the Dish 62 and Orifice 64.

All observations below based upon per ton raw coal washed.

1. Surprisingly, cutting the percentage of solids from 20% to 15% increased wear at velocities of 15 to 24 feet per second which are optimal for best washing. A dish-orifice unit 60 at 13% to 15% solids is replaced every 5,000 tons. Accordingly, a complete study that wear went from a maximum to a minimum starting at about 17% and rising only slowly to 30%. There are at least three factors at play, the cushioning effect starting at about 17%, the water saving effect which increases rapidly between 20% and 30% and the rapidly rising energy requirement for pumping such thicker slurries. With a given low cost pump which is relatively low cost because of its use of a lower horse power electric motor for pumping, the pumping limit governs the cost of the installation. No pump can be used for more than about 80,000 to 100,000 tons without rebuilding or replacing the impeller and housing which are known to wear out quickly.

The optimum solids pumped at low cost is between 18% and 25% and best results were found at 19% raw coal solids in the slurry ( $\frac{3}{4} \times 0$ ). The pump was used for 100,000 tons. The pump was a  $10 \times 8$  low cost Allis Chalmers centrifugal impeller pump with 100 HP rating.

At a pump cost three times greater, an iron ore slurry pump can be used and this lasted a much longer time. The dish-orifice unit 60 which was used with the slurry at about 17% to 20% solids was replaced after 9,000 tons were processed.

(a) Particle Size for Most Efficient Washing

Lowest wear is at particle range  $\frac{1}{2} \times 0$ . At  $1 \frac{3}{4} \times 0$  gouging out of the rubber lining was observed by the large particles. As the particle size was reduced to  $182 \times 0$ , the gouging disappeared and the wear zone was more uniform in appearance and resembled a sand blasted area confined in the dish-orifice unit 60 with the most severe wear occurring in the dish 62 and orifice 64 throat Q, tapering off to a no-wear zone in the cylindrical portion of the orifice 65. No observable wear occurs at the upper lip of the dish 62.

Equally important to efficiency of operation and quality of clean coal is fracturability, sulfur content and ash content of the coal. To properly understand wear, keeping in mind adjustments for fracturability of particle size for high mineral ash content and high inorganic sulfur content, attention to Table A, Section II, is invited.

With all parts in best adjustment and the vortex finder above the 0.00 top edge limit identified in the Table, which is above the top edge of the dish at 0.23B, and with optimum diameters for sleeve D set at 0.36B, orifice E set at 0.21B, in an 18" cyclone, and with dish orifice unit of height H set at 0.69B, wear is monitored at three critical dimensions, as follows:

| Letter | Part                       | Value |
|--------|----------------------------|-------|
| M      | Throat diameter of orifice | .39B  |
| E      | Smallest inside dia-       | .21B  |

-continued

| Letter     | Part                                                                                                          | Value |
|------------|---------------------------------------------------------------------------------------------------------------|-------|
| $\theta_9$ | meter of orifice<br>Included angle of<br>orifice between<br>radius 12 and small-<br>lest inside diameter<br>E | 12°   |

Wearing away of the cyclone parts at the above specified dimensions and identified in Table A contributes the greatest change in percent of recovery and clean coal quality due solely to wear.

Due to the difficulty of directly monitoring  $\theta_9$  and M, the change in E, described in (C) above, is sufficient to reproducibly predict the outside limits of wear which control the efficiency of performance of the cyclone. Thus, subsection (C) above establishes confidence limits of the order of 5% to 6% in projecting wear data with respect to  $\theta_9$  to M. Further, a projection "along the way" can be made because the last  $\frac{1}{3}$  of wear does greater damage to the maximum performance, which is set at "no wear".

#### Quick Change Vortex Finder Sleeve Kit For Maximum Quality and Recovery of Clean Coal

##### (A) Introduction

Each of FIGS. 3, 4, 6, 7, and 8 show different diameter settings of the vortex finder sleeve; the change in diameter D is facilitated by the quick change plate 32 and pivotable fixture bolt 38' which drops the dish. Different dish-orifices 60, 60a, 70, 80 or 90 can each be quickly checked after being dropped and pivoted for wear and then exchanged if need be at the same time when changing the vortex finder sleeves 46, 146, or 246 to the desired setting.

Streamline non-turbulent flow must be maintained (see Case I) in order for high production and efficiency to be achieved in a single, a two stage, or a multi-stage operation beyond two stages. To ensure efficient operation the vortex finder 44 settings, and selection of the dish-orifice 60, 60a, 70, 80 or 90 materials are adjusted to the wear conditions encountered and these must all be handled quickly by means of the quick change plate 32, the fixture bolt 38' and the fasteners 38.

In the fine and coarse coal separation of Case I-IV, Ser. No. 973,408, the most serious problems which were encountered were the quick change steps to maintain high production and efficiency. These changes were specifically:

1. Quick change of diameter settings of vortex finder 44

2. Replacement of different size or worn dishes

An additional problem encountered during the test runs was the optimum vortex finder depth setting. Different raw coals vary in grindability or fracturability as illustrated in Table D, section 6. The crushed particles of dirt and clean coal from easily fracturing coal display large differences between coal and refuse in specific gravities of the order of 0.9 sp. gr. and larger. The more difficult fracturing raw coals produce particles of dirt, low grade middling coals, and clean coals. The middling coals which contain inorganic sulfurs, shales, clays, and other impurities have specific gravities in the range of 1.4 to 1.7. These narrow differences in sp. gr. of about 0.3 units are accounted for by the clinging con-

centration of impurities which do not separate from the clean coal in the coal particle.

The middling coals create the need for a very selective separation process. By very laborious and time consuming testing the importance of the heavy particle spin out was discovered and controlled by the depth of the vortex finder sleeve 46, 146 or 246 bottom edge with respect to the top edge of the dish 60, 62a, 70, 80 or 90.

(B) Criticality of Vortex Finder Height

My first tests in attempting to fix the vortex finder height indicated that the inner swirling upwardly moving clean coal slurry picks up some heavy specific gravity particles which then spin back out of the upwardly moving spiral (the inner spiral and into the downwardly moving spiral (the outward spiral) surrounding the inner swirling upwardly moving spiral path which contains the clean coal. The vortex finder height was changed from a negative value (indicating protrusion into the dish) in a series of trial and error steps to a value that no longer yielded a better quality clean coal. At the value of 0.24 B above the dish edge the maximum improvement in coal quality was discovered. Adjusting the height dimension to a greater value than 0.25 B increased the path of travel of the clean coal particles thus requiring more energy to maintain the vacuuming area and the centrifugal forces necessary to produce efficient separation.

Adjusting the height dimension to a smaller value than 0.22B cut short the heavy specific gravity particle spin out path before the particle had spun to the downwardly moving outer swirling flow thus misplacing the heavy specific gravity particle with the clean coal, thus producing lower quality clean coal. Thus, the height range is 0.22B to 0.25B, preferably 0.23B for optimum performance.

##### (C) Vortex Finder Sleeve Kit

The vortex finder sleeve kit shown in FIGS. 2, 3, 4, 6, 7, 8, 13, 14, 15, 17, 18, and 19 is used to control recovery and improve quality. The height of the vortex finder in relation to the top edge of the dish is set at about 0.23B as pointed out above. The diameter of the vortex finder sleeve is set at about 0.3 B to 0.5 B depending on quality and quantity of clean coal desired. The length of the sleeve 46, 146, 246 in FIGS. 2, 3, 4, 6, 7 and 8 is at least about 0.33 B and is fixed for all sizes because the length serves to stabilize the edges in the vacuum zone.

##### (D) Vacuuming Diameter and Column

The length of the vortex finder sleeve fixed at 0.33 B and height setting of the vortex finder sleeve fixed at 0.23B determine the reverse flow path and the distance that the light sp. gr. particles must travel before exiting out through the sleeve. A length of vortex finder sleeve greater than 0.5B is cumbersome to handle and weld and wasteful of material. The length of the vortex finder sleeve stabilizes the vertical whirling ascending spiral in a fashion to shape it in a constant three dimensional form which is similar to a bell in shape. The diameter of the vortex finder sleeve determines the bottom vacuuming diameter and column of the bell shaped vertical form.

The larger the bottom vacuuming diameter of the bell shaped spiral then the lower the centrifugal force of each particle entering that larger diameter of the bell shaped form. The smaller the bottom vacuuming dia-

ter of the bell shaped vortical the higher the centrifugal force of each particle entering that diameter.

In the dish zone the particles swirling down through the cyclone dish and bottom orifice experience about a threefold increase in Rad PS between the dish top edge and the throat top M of the dish 62, 62a, 72, 82 or 92 in FIGS. 3, 6 and 9-11. This angular acceleration increases the centrifugal force on the particles as they travel along the inner surface of the dish and orifice.

(E) Optimum Centrifugal Force

By empirical testing the optimum centrifugal force for separating light sp. gr. particles from heavy sp. gr. particles for different run of the mine raw coals and gob piles have been determined indirectly through the sizing of the vortex finder sleeve diameter with respect to the percent recovery, raw coal ash content, clean coal ash content and the size of the bottom orifice diameter which expands or contracts "the lead of the screw", e.g., the swirling flow which presents a screw flight pathway within the dish and orifice unit.

The larger the vortex finder sleeve diameter, the lower the centrifugal force displayed by each particle as it enters the larger vacuuming area created by the vortex finder sleeve diameter D. This yields high recoveries with lower quality clean coal.

(f) Method of Changing Vortex Finder Sleeve Kit From One Diameter to Another

The types of sleeve kits are shown in FIGS. 6, 13, and 17. The different size diameter sleeves 46, 146 and 343 are made up from "donuts" cut from steel plate. "Donuts" of different inner diameter are used for insertion of corresponding size sleeves with the sleeve being welded to the "donut". The sleeves have a minimum length of about 0.3B and are made from tubing which is mechanically drawn over a mandrel. Different diameter sleeve kits are shown in FIGS. 2, 3, 4, 5, 7, 8, 13, and 17.

Two types of sleeves can be produced. One, shown in FIG. 4, is a quick-change sleeve 46 with bayonet attachment of the type shown in U.S. Pat. Nos. 795,338 and 1,329,141. The second is the tack and stitch weld attachment sleeve 146 and 246 shown in FIGS. 7 and 8.

In a small cyclone, the tack and stitch weld 152 or 252 can be made through the bottom of the cyclone despite access difficulty by the mirror weld method. This tack and stitch method requires attaching vortex finder sleeves 146 or 246 from the bottom by means of a mirror to aid the welder visually as he tack welds the sleeve in place. This prevents the welder from exposing his body to the hot slag and sparks falling from the welding. Only three stitches or tacks 152 or 252, approximately  $\frac{1}{2}$ " to  $\frac{3}{4}$ " long and equally spaced around the periphery of the vortex finder 144 or 244 and ring 150 or 250, as shown in FIGS. 7 and 8, are required.

Due to the longer change time required for the tack and stitch welding method, bayonet quick-change sleeve 46 is the preferred kit. The plant is able to continue operation with the bayonet modification under any emergency. However, the change sleeves in FIGS. 7 and 8 can be made up in advance, are lower in cost, and can be used when large tonnage of a straight run of mine coal is to be washed. The steel sleeves last for at least 30,000 tons and change is a minor operation during routine maintenance.

Critical Geometry of One Piece Shallow Bottom Dish-Orifice Unit

(a) Relation of Dish-Orifice Unit Depth L to Bowl Diameter B and to Total Bowl Height K

As shown in Table A Section II, the optimum value dish orifice unit depth L expressed in terms of bowl diameter B is about 0.93B, about 17/18 of the bowl diameter. If the depth L is less than about 14/18, e.g. about 0.078 B, then the dish is so shallow as to cut the number of helical turns 170 by about 40% which results in a totally insufficient separation because of a prohibitive reduction of residence time. Further, the upward adjustment of the vortex finder sleeve which is needed to maintain vacuuming dynamics comes dangerously close to the inlet tube level thereby creating the condition which Fitch Jr., et al. claims in U.S. Pat. No. 3,501,014 at Col. 6, lines 59-60 the "short circuit effect" by "contaminants from the inlet to the vortex finder" At L values higher than B, the path 170 in FIG. 6 becomes too long losing energy and separation efficiency. Accordingly, the range of L is 0.82 to B with optimum at 0.93B.

In terms of K, the value of L can best be explained in terms of the effect observed with the path 170 in FIG. 6. Obviously, the deflector created streamline flow providing the three turns of the helical path is clearly dependent upon the total height—e.g. K. By lengthening K to add two or three turns in the upper bowl section above the dish we obviously lose energy. After thousands of observations it was established that two turns are insufficient for separation and more than four turns are wasteful of centrifugal energy which is the sole force used in separation. This results in a K value between 1.12 B to 1.32 B, preferably 1.22 B. Obviously this describes a squat cyclone.

(b) Dish and Orifice Geometry, Vortex Finder Sleeve Area and Orifice Outlet Area

For high speed laminar flow squat cyclones no tight or fast turns in flow direction can be applied to the slurry path yet the path of travel must be a minimum. See FIG. 6. The circular diameter of the swirling flow must be decreased as rapidly as possible without loss of energy, or without turbulence being introduced. Smooth transition curves must be used between included angle changes in geometry, See Table A. Tests to date, indicate that a maximum included angle of 110° is the largest useable dish angle for best separation efficiency. The long cone cyclones experience too great a loss in rotational energy to yield the energy necessary in the separation zone and in the inner upwardly traveling vortical swirl for maximum efficiency. The path distance for particles in a long cone cyclone is at least 3 to 1 compared to the path distance in the cyclone of the invention which indicates a need for three times the energy requirement or only  $\frac{1}{3}$  the energy is available for the separation process.

(c) Identification of Dish Top Angles in Dish Types

The double or single top angles of the dish, indicated by  $\theta_4$  and  $\theta_5$  (for the double angle), or by  $\theta_6$  (only in the single angle) See FIGS. 9, 10 and 11 provides the first compression rotational acceleration increasing the centrifugal force on each particle.

The spiral path through angle  $\theta_5$  continues the speed up process to increase angular velocity accelerating the

rotation expressed in RadP.S. two to three fold. Acceleration of the vertical downward velocity without substantially lessening the kinetic energy and horizontal velocity component results in an increase of the exiting velocity of the refuse from the dish out of the orifice 64a in FIG. 6, where it enters into the top part of the orifice. The separation zone is at the throat of 64 where the height of radius 12 in FIG. 6 is less than one complete spiral height. This fixes separation at the position of the accelerated spiral 170, FIG. 6 at the smallest diameter of 10 the cyclone radius 12 connecting the dish to the orifice.

As shown in FIG. 6, the helix 170 expands at its bottom to increase in height so that in the orifice the helix 170 stretches to occupy the entire throat height T (See Table A) during one revolution. This finish point of this 15 one turn brings refuse to a position at the back of the orifice throat.

The smaller the vortex finder sleeve diameter, the higher the centrifugal force as the particle enters the smaller vacuuming area and lower recoveries with better quality clean coal results.

It is totally unexpected that a shallow dish whose accelerating effect on the downward velocity component exhibits a stabilizing effect on the upward reverse vertical flow of the light particles under vacuuming 25 forces. Stabilization by means of the vortex finder sleeve height 0.033B axially aligns the ascending vortical whirling helix transport light particles along the central axis of the cyclone, and out of the clean coal outlet.

After testing every possible position of the vortex finder in and out of the dish and at the extreme top position in scores of plant runs and in combination with every variation of vortex finder diameter D and orifice diameter E and dish exit diameter M it was discovered that only the critical shallow dimensions in Table A coupled with the vortex finder D dimension constitute the required adjustments for sulphur and ash removal of raw crushed coal. Equally surprising is the discovery that the practical washing of coal having 45 to 50% of 40 ash in a size as large as  $\frac{1}{4} \times 0$  can be carried out successfully based upon this adjustment. Although it is preferable to use smaller crushed sizes e.g.  $\frac{1}{8} \times 0$  or  $\frac{1}{2} \times 0$ , the adaptability of the invention extends to larger sizes for which there is a greater demand for fluidized bed in gas 45 conversion processes.

(d) Bottom Orifice Outlet Diameter E (See Table A)

The existing refuse slurry coming out of the orifice 65a makes an angle of approximately 30° from the horizontal on the right side of the orifice and approximately 45° angle on the left side of the orifice with a left hand spiral within the cyclone. By knowing the lead of the spiral 170 which is controlled by the bottom orifice outlet 65a diameter E, it is possible to determine the 55 path 170 of each particle.

(e) Stages of Separation Double Top Angle  
Dish-Orifice FIGS. 3, 6 and 9

The reduction in diameter within the dish from top to bottom is in a ratio of about 3 to 1. This reduction occurs in a squat cyclone as defined under (a) above having approximately the same height of cylindrical portion as diameter (range of 0.82 to 1.0 of the L/B).

The preferred shortest vertical component of the 65 short path distance is about 0.66 B e.g.  $\frac{1}{3}$  of diameter B of the cyclone. Obviously the descending spiral path 170 provides a longer distance which can be calculated

but is not necessary because the spiral path which is exclusively controlled by the velocity component of the incoming stream and the inlet deflector angle in my copending application Ser. No. 860,330, defines the entrance geometry at the dish e.g. cyclone cylinder parting line and the initial slurry compression by the downward spiral path 170 accompanied by change in spiral path. The transition must be smooth and the change in the inward direction must be gradual since heavy particles in the outer path are at their maximum velocity and it is essential that they maintain their outer position.

The heavy particle travels about 1/10 to  $\frac{1}{8}$  of the diameter and 1/7 of its downward path to lie within an included angle of about 85° at the end of this  $\frac{1}{8}$  distance thereby assuring that there is no changes in lanes as the next or second stage of travel by the heavy particles is entered.

In the second stage representing an additional vertical depth of about 1/7 of the total depth, the heavy particles undergo gradually increasing rate of centrifugal force by an increased spiral velocity in RPM due to the reducing dish diameter. In this second stage where the spiral travels an additional 1/5 of the vertical distance of the total depth of underflow, the gradual change in angle at the lowest point by the second stage reaches about 110°.

Effectively the first stage is a guidance stage of the compound curvature effecting initial gradual passage 30 into the underflow under the angle of 85° for a travel of about 1/5 of the underflow depth. The second stage is an accelerator guidance stage for an additional vertical distance increase of the spiral of 1/7 of the diameter and an added 1/5 of the depth thereby permitting the final 35 or third stage of passage for the spiral at the orifice 64a, FIG. 6.

In the third stage the spiral has diverging paths in about  $\frac{1}{8}$  of the depth to traverse rapidly it would be expected that best results would be achieved by still maintaining this gradual change, however, as pointed out above, the diameter at the second stage exit is about  $\frac{1}{3}$  of the diameter of the dish and it is essential that a final orifice diameter of 1/5 of the dish be attained, which requires that the diameter be cut by about half.

Rather than extending the diameter reduction through the remaining  $\frac{1}{8}$  of the height of the outflow path, the inventor has found it to be essential to create about 100° reduction in the included angle at the throat entering the orifice in a portion of the total underflow height of about 1/5th.

The spiral path, which leaves the critical throat zone of compound curvature of the orifice 64a, FIG. 6, has a cylindrical straight outlet portion (10° to 15° included angle taper) of the orifice which is about only 36% of the underflow thereby leaving about  $\frac{1}{8}$  of the last stage path of about  $\frac{1}{2}$  of the total underflow.

The 100° change in included angle between  $\theta_5$  or  $\theta_6$  and  $\theta_9$ , FIGS. 9, 10 and 11, which is so critical and is mentioned above was determined after production and testing about 15 to 20 test runs of about 6,000 to 8,000 tons each and after painstaking examination of wear patterns on various impact resistant dishes and orifices followed by confirming operational analysis and computer analysis.

The total tonnage which has been run to date and which confirm the above observations is about  $\frac{1}{4}$  million tons and the coal samples have undivided waste coal (gob pile), met coal, steam coal, and sub-bituminous

coals. It's expected that by year end the total tonnage will be above  $\frac{1}{4}$  million.

(e) Separation in Single Top Angle Dish of FIGS. 10 and 11

More specifically, the unit has five distinct zones. The top entrance zone has a  $\frac{1}{8}$  inch wide top radius lip that contacts the bowl wall and directs the swirling flow from a zero included angle through an  $80^\circ$  included angle change, to a  $100^\circ$  included angle making one continuously straight cone surface along a center line distance of  $0.23 B$ . At this depth the swirling flow is directed, by a  $0.194 B$  radius 12 along the smooth surface through another continuously changing angle reducing to  $100^\circ$  included angle to a  $12^\circ$  included angle via a center line distance of  $0.14 B$ . The swirling slurry is at a depth of  $0.38 B$  as it begins its path along the conical surface which forms the  $\theta_9$  included angle along a center line path of  $0.25 B$ . The total depth of the dish and orifice unit at the bottom of  $\theta_9$  included angle surface is  $0.63 B$ . At this depth the swirling flow is directed through the last included angle change of about  $12^\circ$ . The swirling flow diameter has been reduced from  $B$  diameter to about  $0.20 B$  diameter in a center line distance of  $0.63 B$ . The  $0.06 B$  center line distance the flow travels in its last straight walled cylinder yields a slower wearing diameter  $E$  thus reducing the rate of change of the smallest diameter at the end of the unit.

The above geometry is used for the ceramic ( $Al_2O_3$ ) dish and orifice unit 92, FIG. 11, to minimize manufacturing cost. The important geometry is that of reducing the diameters at a set rate in the different zones of the unit to preserve smooth streamline laminar flow. The first diameter reduction via a straight walled cone from  $B$  to  $0.39 B$  along the center line distance of  $0.24 B$  is maintained. The remainder of the unit is identical to the other one and two piece units tested.

The aluminum oxide ( $Al_2O_3$ ) dish and orifice unit can be substituted for the urethane and other wear resistant dish and orifice units to take advantage of the wear characteristics of ( $Al_2O_3$ ). All of the different material dish and orifice units will perform well on all slurries, but with different rates of wear. The selection of different materials for the dish and orifice unit makes available parts of different costs to satisfy any policy on inventory.

Raw Coal Particle Size, Mineral Impurity Hardness and Effect on Recovery

(A) Crushed Raw Coal Particle Size

It is known that mined coal must be crushed for liberation of mineral ash, inorganic sulfur, and other coal impurities. Cleaning differences were observed in raw coals of different fracturability crushed to the same size and having the same raw percent of ash and sulfur, yet processed with the same plant settings. Raw coals producing the heaviest load on the plant sizing screens and requiring maximum energy for crushing the coal by the coal crusher yielded the poorest quality clean product. It was further discovered that harder coals required smaller sizings, e.g., lower particle sizes, to yield the product that softer raw coals produced, the optimum size being  $\frac{1}{2} \times 0$ . Softer coals do not overload the screen and crushers and the refuse is different from that of harder coals. The settings are shown in FIGS. 23 24 and 25 illustrating the different values required for harder coals and for softer coals for  $\frac{1}{2} \times 0$  coal size.

(B) The Influence of Primary Mineral Impurities in Crushed Coal on Washing Efficiency

(1) High Ash in Hard Coal—Identification by Mineral Hardness on Moh's Scale and Upper Freeport Seam

The optimum size in the invention at  $\frac{1}{2} \times 0$  for hard coal can be extrapolated from FIGS. 23, 24 and 25 and it is only necessary to use the "top coal", first stage curve in FIG. 23.

The primary hard minerals associated with coal are quartz (hardness, H7), garnet (H7-7.5), topaz (H8), tourmaline (H7-7.5), zircon (H7.5), augite (H5-6), and rutile (H6-6.5). These give problems during grinding of the coal. The principal materials of coal such as vitrinite, exinite, fusinite, and inertinite are easily fractured. However, the presence of 15 to 25% mineral ash makes certain coals very difficult to fracture. An example is in the Upper Freeport Seam. It is not the quantity of the ash but the quality of the ash which governs fracturability. Coal from the Upper Freeport Seam taken below the Big Joe binder is very difficult to grind. The grindability on the hardgroove grindability index is about 80.6 which represents a much less fracturable coal than the standard. The Big Joe bottom coal had an ash of about 22 to 30% in the run of the mine. The seam is shown below.



## (2) High Ash in Soft Coal and Gob Pile, Georges Creek

Another example of Gob pile coal from Georges Creek, Lonaconing, Md. which is low in sulfur and was believed to be unwashable for about 100 years has an ash content of 25 to 40% with a sulfur of 0.70 was the most friable and easily fractured material of high ash content which the inventor has ever handled.

In the 3 cyclone preparation plant, the inventor could grind and wash 150 TPH of Gob pile but with difficulty and great care could wash only 90 TPH of Big Joe bottom coal due to overloading the sizing circuit of the plant. Accordingly the maintenance of highest standards for production of clean coal quality at minimal plant investment requires careful attention to the fracturability of the coal being washed. Obviously, a more expensive crusher adapted to fracture harder materials can be used but this would increase the cost of the plant.

## (C) High Inorganic Sulfur, Wheelock Recommendations

In the ACS Symposium Series of Coal Desulfurization Chemical and Physical Methods, by Thomas D. Wheelock, copyright 1977, it is stated, at page 37, that "removing sulfur from coal requires reducing the particle size of the coal prior to direct physical separation with water washing": The author of this section, J. A. Cavallaro et al described crushing (Lower Freeport Bed Coal and Pittsburgh Bed Coal) to 200 mesh, both samples being taken from mines in West Virginia. The Lower Freeport Bed sample gave maximum reduction in pyritic sulfur for the 14 mesh (about  $\frac{1}{4}$ ") fraction. It is of interest to note that the Lower Freeport sample is similar to the Upper Freeport Seam tested by the inventor and sulfur content is comparable. The Pittsburgh bed gave maximum sulfur reduction at 48 mesh. Grinding the Lower Freeport sample down to 200 mesh gave little improvement. Grinding the Pittsburgh sample from 48 mesh to 200 mesh gave little improvement.

In contrast to Wheelock, the present invention uses much coarser particle sizes. Some coals are cleaned at  $1\frac{1}{2} \times 0$  and cleaning is even better at  $\frac{3}{4} \times 0$ . The best quality is in the particle size range of  $\frac{1}{2} \times 0$  so that all coals can be washed and down time for changing size can be avoided.

Below the inventor proposes a relative fracturability index at a scale from 0 to 10. 100 is the grindability of coal from the Jerome Mines, Upper Kittanning Bed. This 100 value is assigned a relative fracturability index of 0 in the inventor's index, see Table C below.

TABLE C

| Relative Fracturability Table |                        |
|-------------------------------|------------------------|
| Relative Fracturability       | Hardgrove Grindability |
| 1                             | 97 $\frac{1}{2}$       |
| 2                             | 95                     |
| 4                             | 90                     |
| 6                             | 85                     |
| 8                             | 80                     |
| 10                            | 75                     |

## (D) Sulfur Removal in Presence of Clay

If the particles are very large so that the heavies are not exposed as separable particles, then coarser particles can contain washable coal and may be lost. These coarse particles must be reground to finer size and re-washed.

After washing several dozen different types of coal of different grindabilities containing high sulfur and difficult to remove clays, it was found that it is not economical to wash below 5% mineral ash (on a dry basis) and that it is not possible to wash out organic sulfur with water only.

The same experience is found in larger scale plants such as the jigging cyclone plant installed by McNally Pittsburgh at Wilson, Md. The coal for jig washing is at a size of  $\frac{3}{8} \times 0$  in order to get the practical low particle size for sulfur removal.

## (E) Fracturability of Raw Coal in Terms of Hardgrove Index

The grindability of a coal is a measure of ease of pulverizing that coal compared to the ease of pulverizing of a standard coal that has been assigned a Hardgrove Index of 100. The standard coal is a low-volatile coal such as that from the Jerome Mines, Upper Kittanning Bed, Somerset County, Pa. Thus a coal with a grindability of 125 could be pulverized more easily than the standard while a coal with a grindability of 70 would be more difficult to grind. The Hardgrove Index is defined in Chemical Engineers' Handbook, 5th Ed., pgs 8-8 and 8-52.

## (3) Correlation in FIG. 23 between Ease of Fracturing and Quality of Clean Coal Produced

Reference is made to FIG. 23 wherein the curve for "Big Joe Coal" takes into account fracturability by crushing raw coal to a size of  $\frac{3}{8} \times 0$  in the cyclone washing plant of the present invention in the 18" cyclone. FIG. 23 shows the percent of ash removal in a range of 10% ash to 100% ash removal on the x axis and the percent top recovery on the y axis. Comparing Big Joe and Top Coal in the two curves of FIG. 23 gives the difference in percent recovery based on fracturability.

## (F) Screening Followed by Crushing (Rotary Breaker) and Second Screening and Crushing Steps

Incoming coal is first screened in a primary screen before passing through the rotary breaker. A secondary screen using about  $\frac{1}{2}$ " square screen cloth is then used to screen the coal from the breaker and primary screen to constitute the raw coal feed before it enters the first stage slurry tank.

The primary screen and rotary breaker are equipped with  $1\frac{1}{2}$ " screen cloths which results in the feed into the breaker being broken into sizes of  $1\frac{1}{2}$ " minus. All lumps that do not break while in the rotary breaker are discharged to a refuse pile. All lumps that break into sizes of  $1\frac{1}{2}$ " minus are circulated into the other  $1\frac{1}{2}$ " minus size circuit from the primary screen and are fed to the secondary screen where all the feed is then sized into two fractions.

One fraction passes through the  $\frac{1}{2}$ " square screen cloth and is discharged into the first stage slurry tank. The other fraction is fed into the coal crusher where it will be crushed to size and recirculated back across the secondary screen to insure that any oversize particles are not discharged into the first stage slurry tank.

## Examples of Critical Location of Cyclone Parts

## (A) Wear in Cyclone Head Space FIGS. 3 &amp; 6, 7 &amp; 8 Between Plate 30 and Inlet 22

The inventor has found that any space between plate 30 and inlet 22 within the cyclone bowl 28 is a very

abrasive zone. This suggests disrupting unstreamlined flow and for this reason an abrasive resistant spacer plate 30 is fitted to the top cover plate 29 of the cyclone 20 to fill this void. The inlet 22 can be raised to the top for cast cyclone 20 inlets 22 and top portions that do not represent any undo manufacturing difficulties.

(B) Criticality of Cyclone Height L

As mentioned in Section V, the energy in the inner swirling upwardly moving spiral flow derives from the amount of energy contained by the downwardly outer moving swirl at the separating zone within unit 60, 60a, 70, 80 or 90 downwardly outer swirl has a greater distance of travel, the energy loss proportional to distance, reduces the centrifugal energy upon entering the separation zone and the inner upwardly moving swirl has less energy.

(C) Example of Plant Settings

(1) Two Stage Washing

If it is desirous to clean 13% ash raw coal of a suitable fracturability to produce met coal of 8% ash or less and 1.15 or less % sulphur, it would require a two stage plant setting of 661/2% cyclone top % recovery in the first stage, see FIG. 12 of my co-pending patent application Ser. No. 2,731, and a 43% cyclone top % recovery in the second stage, reference to FIG. 12. This would yield an 81% plant recovery of met coal.

A 0.35 B" diameter D vortex finder sleeve 46, 146, or 246 coupled with the 0.21 B" inside diameter E orifice containing the  $\theta_9$  included angle and the 0.19 B radius connecting throat top M to  $\theta_9$  installed in the first and second stage will yield the above setting. Now the cyclone top % recovery will slowly drop off as the 0.21 B diameter E is worn out to 0.22 B".

At a 0.22 B" diameter E the cyclone top % recovery for the coal described and the 0.35 B" diameter D vortex finder sleeve, 46, 146 and 246, would be 50% for the first stage and 26% for the second stage yielding an overall plant % recover of 63% thus a loss of 17% misplaced material. The 63% recovery will still meet met specifications but the 17% loss will warrant new orifices.

The amount of wear tolerated will depend on the coal being processed. As an example a new set of orifices 64, 45 64a, 74, 84 and 94 could be used for producing a high recovery rate for say met or steam coal from a specific raw coal and then when they have worn to a new recovery setting (See FIG. 14 of my co-pending patent application Ser. No. 2,731) a raw coal could be processed that requires the worn geometry.

The only critical part involved in the wear is that it is even and doesn't produce uneven surfaces that will cause turbulence. When this occurs the orifices 64, 64a, 74, 84 and 94 must be replaced. The  $\theta_9$  included angle and the 0.19 B" radius between throat top M and  $\theta_9$  produces an even wearing orifice 64, 64a, 74, 84 and 94 and at the same time it will maintain the smooth laminar flow required for efficient ash and pyritic sulphur removal.

It is critical that the wear pattern be controlled to maintain the internal geometry of  $\theta_9$  included angle and 0.19 B" radius between throat top M and  $\theta_9$  throughout the useful life of the orifice 64, 64a, 74, 84 and 94 to not cause disturbance in the flow pattern so as not to disrupt the centrifugal separation process occurring within the throat of the orifice. A change in the included angle can cause the separation process to raise out of or lower into

the throat thus producing a different ash and pyritic sulphur removal efficiency.

(D) Single Outlet and Multi Stage Plant

5 Set the first stage to recover only high premium coal with some of this coal escaping to the first stage refuse stream and being recovered in the successive stages of washing.

10 For all around plant performance washing many different types of raw coal feed, the centrifugal separator cyclones proved to have the best operating efficiencies when set at 35% top recovery for very high ash raw coal feeds, e.g. 35% ash and higher, to 65% top recovery when washing very low ash raw coal feeds e.g. 11% to 16% ash. For washing raw coals in between these qualities requires adjustments accordingly.

15 Reference to FIG. 14 cyclone recovery graph of my co-pending patent application Ser. No. 2,731 for correct settings when washing different raw coal feeds is made.

20 One will note that this graph gives the vortex finder sleeve diameter and area, the bottom orifice diameter, the raw coal feed % ash, and the cyclone top percent recovery. This graph does not tell you where the plant should operate to produce a certain quality coal.

25 Graphs F.12 ash removal and F.13 Inorganic sulphur removal must be used first to determine what cyclone top percent recovery will be required to produce the quality coal desired. As an example let's suppose we will be seeking a metallurgical coal quality having the following specifications:

Clean Coal

30 1. % ash 8.0 or less  
2. Total % sulphur 1.0 or less  
3. and other metallurgical qualities, free swelling index, etc. and the run of the mine raw coal feed has the following specifications:

Raw Coal

35 1. % ash 14.0 average  
2. Total % sulphur 3.0 average  
3. % Organic sulphur 0.5 average with the remainder being inorganic sulphurs  
4. and other metallurgical qualities, free swelling index, etc.

Plant Settings of an 18 Inch Cyclone

How should the cyclones be set to produce a metallurgical coal? Graph, FIG. 12 of my co-pending patent application Ser. No. 2,731, ash removal, which was produced over a period of 100,000 tons of coal washed, shows two curves for the first stage settings. One curve is labeled Top Coal and the other Big Joe Coal. The major difference in these two coals is the crushability. The Top Coal crushes very easily to size. The Big Joe coal is very difficult to crush. It is assumed that, if the Big Joe Coal is crushed to the same size, e.g.,  $\frac{1}{2}'' \times 0$ , as the Top Coal, it will then have the same curve as the Top Coal. Since our example coal can be crushed to the correct size, we use the Top Coal curve. The question now arises as to how much ash removal is required to produce a metallurgical coal, e.g., 7.5% clean coal percent ash. Based upon past experience, a first setting of 60 cyclone top percent recovery is at 60%.

65 Following the 60% line horizontally to the right until it intersects the first stage Top Coal curve and then following this intersection point vertically down the

graph, this line intersects the percent ash removal axis at 68%. Now check to see if this percent recovery and percent ash removal will produce the metallurgical coal desired. Using a two stage centrifugal separator cyclone coal preparation flow chart, the check is made.

#### Tonnage Targets and Quality Control

When 150 tons are fed to the plant and 60% by weight is recovered in the first stage with 68% of the ash removed, then the first stage produces 90 tons of clean coal yielding a 7.47% ash clean coal. The first stage refuse consists of 60 total tons of which 14.28 tons are ash. This gives a 23.80% ash raw coal feed to the second stage.

The sulphur quality must now be checked. 60% cyclone top percent recovery corresponds to 90% inorganic sulphur removed using F.13 Inorganic Sulphur Removal graph of my co-pending patent application Ser. No. 2,731 produced over a period of 100,000 Tons of coal washed.

The first stage clean coal sulphur content prediction is:

Inorganic sulphur wt.—0.37 tons  
Organic sulphur wt.—0.52 tons  
% Inorganic S<sub>2</sub>—0.41  
% Organic S<sub>2</sub>—0.58  
% Total S<sub>2</sub>—0.99

The first stage refuse sulphur content prediction is:

Inorganic sulphur wt.—3.38 tons  
Organic sulphur wt.—0.23 tons  
% Inorganic S<sub>2</sub>—5.63  
% Organic S<sub>2</sub>—0.28  
% Total S<sub>2</sub>—6.01

#### First Stage Clean Coal Settings

The first stage clean coal quality prediction meets the metallurgical coal specification so the next step is to set the cyclone dimensions. With the cyclones operating at correct pressures, % solids, and flow velocities, e.g., 23 psi, 19%, 22 FPS, the dimensional settings from F.14 Cyclone Recovery graph of my co-pending patent application Ser. No. 2,731 to produce 60% cyclone top percent recovery are:

1. Fixed 3 $\frac{5}{8}$ " bottom orifice diameter with correct dish and orifice geometry.
2. Fixed 14% ash run of the mine raw coal feed.
3. 6" inside diameter vortex finder sleeve is installed.

#### Second Stage Washing

The next step is to set the second stage to produce metallurgical coal. The feed to the second stage is the refuse from the first stage. The mixing and pumping of the first stage refuse, that occurs between the orifice outlet of the first stage cyclones and the inlet to the second stage cyclones; breakes, washes, and dislodges from the clean coal particles, tightly bound shales, clays, pyrites and other coal impurities. This accounts for the better separation efficiencies shown on graph F.12 Ash Removal of my co-pending patent application Ser. No. 2,731 for the second stage both coals curve.

#### Second Stage Settings

The first stage refuse is predicted to have the following specifications:

Prod. Weight—60 TPH  
Ash Weight—14.28 Tons  
% Ash—23.80%  
Io S<sub>2</sub> Weight—3.38 Tons

% Io S<sub>2</sub>—5.63% O S<sub>2</sub>—0.23 Tons % O S<sub>2</sub>—0.38%  
% Total S<sub>2</sub>—6.02

We must meet metallurgical coal specification of 7.5% ash so we will look at the % ash first. From experience using F.12 Ash Removal graph 40% recovery will be predicted as correct cyclone top % recovery. This % recovery corresponds to a 87.3% ash removal. The recovered product weight will be 24 TPH containing 1.81 TPH of ash yielding a 7.56% ash clean coal product which is approximately equal to 7.5% ash.

Next the sulfur removal must be considered. The metallurgical specification is 1.0% or less. Using FIG. 12, Inorganic Sulfur Removal Graph of my co-pending patent application Ser. No. 2,731 as the guide, at a 40% cyclone top percent recovery, this will correspond to 96.7% inorganic sulfur removal. The recovered product will then contain 0.11 TPH inorganic sulfur and 0.11 TPH organic sulfur yielding a 0.46% inorganic sulfur, 0.46% organic sulfur and 0.92% sulfur total. The percent ash and percent sulfur satisfies the specifications for met coal. Thus, the setting which are obtained from FIG. 14, Cyclone Recovery Graph of my co-pending patent application Ser. No. 2,731, can be verified in practice.

#### EXAMPLES

##### (A) Example 1

Example 1 of Table D, runs 1A through 7A, are plant production runs. The Upper Freeport coal is from a strip mine located in Preston County, West Virginia. The local stripper calls it his Top Coal. The raw coal analysis varies as indicated by the % mineral ash of the feed and the % sulphur content of the feed, Example 1. This coal has a 2 to 4 relative fracturability index, thus the coal breaks apart easily exposing the pyrites and mineral ash to the centrifugal separation. The results are 83% to 90% of the pyritic sulphur being removed and the mineral ash being reduced well below the 8.5% limit with total product recoveries between 82 and 89%.

The fluctuation in % pyritic sulphur being removed depends on the varying fracturability of the coal which is caused by variations in the small binders of hard shales, hard coals and other mineral ashes. If the pyrites are located along the cleavage lines and if the lumps will break apart along these lines then the pyrites become the easiest refuse to separate because of the high (5.02) specific gravity of the pyrites compared to the lower 2.6 and higher specific gravities of the clays, shales, rock and other contaminating minerals.

The fluctuating fracturability is demonstrated by run 7B in Example 2 of Table D. This particular run demonstrates the fracturability index of the coal lowering. The coals in Example 1 and Example 2 came from the same strip pit. Example 1 is called the top coal, and Example 2 called Big Joe which is a thick hard coal seam. Depending on how selective the mining people are they may mix or else the hardness characteristic fluctuates up and down through the two different coal beds and some of the harder coals may get mixed with the softer coals and vice versa.

##### (B) Example 2

Example 2 run 7B was border line coal that had a relative fracturability index of around 5. It barely missed producing met coal but it made excellent steam coal. This coal helps by blending to reduce the total % sulphur of the other steam coals. It is very conceivable

that if this coal could have been crushed to  $\frac{1}{2}'' \times 0$  that the % total sulphur could have fallen below 1.5 and the ash quality meeting met quality. Example 2 clean coal quality meets the present steam coal order of the stripper's and cleaning plant owner's; thus he didn't want to spend more money and lower recoveries to make the coal a better quality. The most important aspect of Example 2 is the ability to clean Big Joe to meet a consumers specification. Before the present plant was installed this hard binder coal had been disregarded because of not being washable in other known methods. Besides its high relative fracturability index it has a large quantity of clay binders and is difficult to wash.

Other cleaning plant personnel stated that Big Joe coal could not be cleaned because the clays would plug the clean coal dewatering screens and the centrifugal dryer basket screens. With the present invention the clays were no problem. The clays broke out of the coal on crushing and easily separated when exposed to the high centrifugal forces. Because of the complete separation of the clays they reported to the refuse and never came in contact with the clean coal dewatering screens and the clean coal centrifugal dryer basket screens.

(C) Example 3

Example 3, runs 1C and 2C, is coal from a gob pile located near Georges Creek; Lonaconing, Maryland. The gob pile is believed to be about 100 years old. The

of the low sulphur content. This gob will contain a feed mineral ash of from 26% to 40% and a sulphur of around 0.7%. The sulphur content of the clean coal rises, because of only traces of inorganic sulphurs and practically all organic sulphur. This gob separates very easily because of the low present fracturability index of 3 to 5. Before being delivered to the plant the gob is processed through a shaker screen to remove all materials of 2" or bigger top size.

10

(D) Example 4

Example 4, runs 1D and 2D, is a hard binder coal that was separated from the soft good coal, from a strip mine in Somerset County, Pa., by processing the coal through a rotary breaker. The hard binder coal is the refuse from the rotary breaker. This coal has a present fracturability index of 8-9. A stone crusher type crusher is necessary to crush this coal. The feed mineral ash varied between 26% and 35% with a feed sulphur content of 1.0% to 1.1%. This coal produces an excellent low sulphur steam coal. It was used to blend lower quality coal to meet the steam coal market.

15

Example 1 represented 7270 tons; Example 2-7040 tons; Example 3-2400 tons; and Example 4-2400 tons of raw coal processed using the invention. To date, the invention has processed approximately 300,000 tons of various types (different present fracturability index) coals successfully.

TABLE D

| Coal Type      |      | EXAMPLE 1 | Tons of Washed Coal | % Feed Recovered | Metallurgical 2 to 4 LF Index |               |             | Crush Size $\frac{1}{4}'' \times 0$ |               |             | % Mineral Ash Feed | Coal Dry |
|----------------|------|-----------|---------------------|------------------|-------------------------------|---------------|-------------|-------------------------------------|---------------|-------------|--------------------|----------|
|                |      |           |                     |                  | % Pyritic Dry                 | % Organic Dry | % Total Dry | % Pyritic Dry                       | % Organic Dry | % Total Dry |                    |          |
| Run of 8 Hours | Date |           |                     |                  |                               |               |             |                                     |               |             |                    |          |
| 1A             | 5/20 | 851       | 81.82               | 1.70             | 0.80                          | 2.50          | 0.36        | 0.80                                | 1.16          | 14.20       | 7.32               |          |
| 2A             | 5/22 | 878       | 84.44               | 1.16             | 0.80                          | 1.96          | 0.26        | 0.80                                | 1.06          | 15.00       | 7.48               |          |
| 3A             | 5/30 | 908       | 87.28               | 2.30             | 0.80                          | 3.10          | 0.42        | 0.80                                | 1.22          | 15.49       | 7.40               |          |
| 4A             | 5/31 | 931       | 89.55               | 2.27             | 0.80                          | 3.07          | 0.36        | 0.80                                | 1.16          | 15.31       | 7.56               |          |
| 5A             | 6/02 | 855       | 82.21               | 0.96             | 0.80                          | 1.76          | 0.12        | 0.80                                | 0.92          | 13.39       | 6.32               |          |
| 6A             | 6/03 | 870       | 83.65               | 0.96             | 0.80                          | 1.76          | 0.18        | 0.80                                | 0.98          | 11.58       | 5.99               |          |
| 7A             | 6/05 | 895       | 86.05               | 0.86             | 0.80                          | 1.66          | 0.31        | 0.80                                | 1.11          | 14.36       | 8.04               |          |

LF INDEX IS RELATIVE FRACTURABILITY INDEX OF PRESENT LILLER APPLICATION

| Coal Type      |      | EXAMPLE 2 | Tons of Washed Coal | % Feed Recovered | Steam 5 to 8 LF Index |               |             | Crush Size $\frac{1}{4}'' \times 0$ |               |             | % Mineral Ash Feed | Coal Dry |
|----------------|------|-----------|---------------------|------------------|-----------------------|---------------|-------------|-------------------------------------|---------------|-------------|--------------------|----------|
|                |      |           |                     |                  | % Pyritic Dry         | % Organic Dry | % Total Dry | % Pyritic Dry                       | % Organic Dry | % Total Dry |                    |          |
| Run of 8 Hours | Date |           |                     |                  |                       |               |             |                                     |               |             |                    |          |
| 1B             | 5/18 | 756       | 82.21               | 2.17             | 0.80                  | 2.97          | 1.13        | 0.80                                | 1.93          | 18.31       | 11.30              |          |
| 2B             | 5/19 | 734       | 79.75               | 2.91             | 0.80                  | 3.71          | 1.69        | 0.80                                | 2.49          | 17.03       | 10.96              |          |
| 3B             | 5/20 | 738       | 80.27               | 1.92             | 0.80                  | 2.72          | 1.44        | 0.80                                | 2.24          | 15.49       | 9.85               |          |
| 4B             | 5/23 | 704       | 76.49               | 1.84             | 0.80                  | 2.64          | 0.96        | 0.80                                | 1.76          | 17.16       | 9.90               |          |
| 5B             | 5/24 | 730       | 79.34               | 2.37             | 0.80                  | 3.17          | 1.29        | 0.80                                | 2.09          | 17.18       | 12.55              |          |
| 6B             | 5/25 | 713       | 77.51               | 2.49             | 0.80                  | 3.29          | 1.66        | 0.80                                | 2.46          | 20.02       | 12.01              |          |
| 7B             | 6/01 | 646       | 70.17               | 1.50             | 0.80                  | 2.30          | 0.46        | 0.80                                | 1.26          | 17.85       | 8.59               |          |
| 8B             | 6/01 | 717       | 77.95               | 1.15             | 0.80                  | 1.95          | 0.90        | 0.80                                | 1.70          | 19.84       | 12.12              |          |

gob never underwent spontaneous combustion because

| Coal Type      |      | EXAMPLE 3 | Tons of Washed Coal | % Feed Recovered | Steam 3 to 5 LF Index |               |             | Crush Size $\frac{1}{4}'' \times 0$ |               |             | % Mineral Ash Feed | Coal Dry |
|----------------|------|-----------|---------------------|------------------|-----------------------|---------------|-------------|-------------------------------------|---------------|-------------|--------------------|----------|
|                |      |           |                     |                  | % Pyritic Dry         | % Organic Dry | % Total Dry | % Pyritic Dry                       | % Organic Dry | % Total Dry |                    |          |
| Run of 8 hours | Date |           |                     |                  |                       |               |             |                                     |               |             |                    |          |
| 1C             | 9/06 | 713       | 67.04               | Traces           | 0.74                  | 0.74          | Traces      | 0.79                                | 0.79          | 0.79        | 25.72              | 11.94    |
| 2C             | 9/07 | 688       | 66.21               | Traces           | 0.70                  | 0.70          | Traces      | 0.73                                | 0.73          | 0.73        | 26.89              | 11.58    |

COALS 1C AND 2C, EXAMPLE 3, DID NOT MEET FREE SWELLING INDEX TO MET COAL

| Example 4 Coal Type Steam 8 to 9 LF Index Crush Size $\frac{1}{4} \times 0$ |      |     |       |      |      |      |      |      |      |       |       |
|-----------------------------------------------------------------------------|------|-----|-------|------|------|------|------|------|------|-------|-------|
| 1D                                                                          | 9/07 | 643 | 61.87 | 0.21 | 0.85 | 1.01 | 0.10 | 0.85 | 0.95 | 25.81 | 11.24 |
| 2D                                                                          | 9/08 | 635 | 61.24 | 0.24 | 0.85 | 1.09 | 0.10 | 0.85 | 0.95 | 27.34 | 11.59 |

Having thus disclosed the invention, I now claim:

1. A method of water washing crushed coal for gravitational separation in a centrifugal separating cyclone at low speed pumping at a pressure of 8-18 psig between the inlet and the vortex finder outlet, said cyclone having a circular bowl and being fitted with a vortex finder, a vortex finder cylindrical sleeve, a dish, an orifice and a feed pipe, said cyclone having a height to diameter ratio of 0.90 to 0.95, in which light fractions are removed through the vortex finder at the top of the cyclone and heavy fractions pass through the orifice at the bottom, said method comprising:

(a) installing a removable one-piece dish-orifice unit made of erosion resistant material selected from the group consisting of ceramic, refractory carbide alloy, urethane rubber, nickel hardened cast iron and nickel hardened cast steel,

(b) providing the geometry of the dish portion of said dish orifice unit by limiting the height of the dish portion to between 0.15B and 0.67B, where B is the inner diameter of the circular cyclone bowl, and providing a first included angle of the dish at the top edge of 85° within a range of +15° or minus 15° and providing a second included angle of the dish below the first included angle of 110° within a range of +15° and 15° and, the third included angle in the throat of the orifice of 12° with a variation of from plus 7° to 12° to minus 3° which is 9°;

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750

UNITED STATES PATENT AND TRADEMARK OFFICE  
CERTIFICATE OF CORRECTION

PATENT NO. : 4,341,352

DATED : July 27, 1982

INVENTOR(S) : Delbert I. Liller

It is certified that error appears in the above-identified patent and that said Letters Patent is hereby corrected as shown below:

Claim 1, line 22, "+150°" should read --+15°--.

Signed and Sealed this

Twenty-ninth Day of March 1983

[SEAL]

Attest:

GERALD J. MOSSINGHOFF

Attesting Officer

Commissioner of Patents and Trademarks